



US007727421B2

(12) **United States Patent**  
**Hsu et al.**

(10) **Patent No.:** **US 7,727,421 B2**  
(45) **Date of Patent:** **Jun. 1, 2010**

(54) **ELECTRICALLY CONDUCTIVE POLYMER COMPOSITIONS**

(75) Inventors: **Che-Hsiung Hsu**, Wilmington, DE (US); **Sunghan Kim**, Goleta, CA (US); **Ian Storms Moody**, Eugene, OR (US)

(73) Assignee: **E. I. du Pont de Nemours and Company duPont Displays Inc.**, Wilmington, DE (US)

(\*) Notice: Subject to any disclaimer, the term of this patent is extended or adjusted under 35 U.S.C. 154(b) by 855 days.

(21) Appl. No.: **11/475,345**

(22) Filed: **Jun. 27, 2006**

(65) **Prior Publication Data**

US 2007/0045591 A1 Mar. 1, 2007

**Related U.S. Application Data**

(60) Provisional application No. 60/694,276, filed on Jun. 27, 2005.

(51) **Int. Cl.**

**H01B 1/00** (2006.01)  
**C08G 75/00** (2006.01)  
**C08G 73/00** (2006.01)  
**C08G 73/06** (2006.01)

(52) **U.S. Cl.** ..... **252/500**; 528/377; 528/422; 528/423

(58) **Field of Classification Search** ..... **252/500**; 528/377, 422, 423  
See application file for complete search history.

(56) **References Cited**

**U.S. PATENT DOCUMENTS**

3,282,875 A 11/1966 Connolly et al.

|                  |         |                          |
|------------------|---------|--------------------------|
| 4,358,545 A      | 11/1982 | Ezzell et al.            |
| 4,433,082 A      | 2/1984  | Grot                     |
| 4,940,525 A      | 7/1990  | Ezzell et al.            |
| 5,300,575 A      | 4/1994  | Jonas et al.             |
| 5,463,005 A      | 10/1995 | Desmarreau               |
| 6,150,426 A      | 11/2000 | Curtin et al.            |
| 6,303,238 B1     | 10/2001 | Thompson et al.          |
| 6,670,645 B2     | 12/2003 | Grushin et al.           |
| 2007/0069184 A1* | 3/2007  | Hsu et al. ..... 252/500 |
| 2008/0213594 A1* | 9/2008  | Hsu ..... 428/411.1      |

**FOREIGN PATENT DOCUMENTS**

|    |                 |         |
|----|-----------------|---------|
| WO | WO 98/31716 A1  | 7/1998  |
| WO | WO 99/52954 A1  | 10/1999 |
| WO | WO 00/70655 A2  | 11/2000 |
| WO | WO 01/41512 A1  | 6/2001  |
| WO | WO 03/006537 A1 | 1/2003  |
| WO | WO 03/008424 A1 | 1/2003  |

(Continued)

**OTHER PUBLICATIONS**

U.S. Appl. No. 60/105,662, filed Oct. 25, 1999, Zhen-Yu Yang et al.

(Continued)

*Primary Examiner*—Mark Kopec  
*Assistant Examiner*—Jaison P Thomas  
(74) *Attorney, Agent, or Firm*—John H. Lamming

(57) **ABSTRACT**

There is provided an electrically conductive polymer composition, comprising a first electrically conductive polymer doped with an organic solvent wettable fluorinated acid polymer in admixture with a second electrically conductive polymer doped with an organic solvent non-wettable fluorinated acid polymer.

**26 Claims, 1 Drawing Sheet**



## FOREIGN PATENT DOCUMENTS

WO WO 03/040257 A1 5/2003  
WO WO 03/063555 A1 7/2003  
WO WO 03/091688 A2 11/2003  
WO WO 2004/016710 A1 2/2004

## OTHER PUBLICATIONS

U.S. Appl. No. 60/176,881, filed Jan. 19, 2000, Jose M. Rodriguez-Parada.  
Kyunghoon Lee et. al., Poly(thieno[3,4-b]thiophene). A New Stable Low Band Gap Conducting Polymer, *Macromolecules*, 2001, vol. 34:5746-5747.  
Gregory A. Sotzing et. al., Poly(thieno[3,4-b]thiophene): A p- and n-Dopable Polythiophene Exhibiting High Optical Transparency in the Semiconducting State, *Macromolecules*, 2002, vol. 35:7281-7286.

A. Feiring et. al., Aromatic Monomers With Pendant Fluoroalkylsulfonate and Sulfonimide Groups, *Journal of Fluorine Chemistry*, 2000, vol. 105:129-135.

A. Feiring et. al., Novel Aromatic Polymers With Pendant Lithium Perfluoroalkylsulfonate or Sulfonimide Groups, *Macromolecules*, 2000, vol. 33:9262-9271.

D.D. Desmarreau, Novel Perfluorinated Ionomers and Ionenes, *J. Fluorine Chem.*, 1995, vol. 72:203-208.

A.J. Appleby et. al., Polymeric Perfluoro Bis-Sulfonimides as Possible Fuel Cell Electrolytes, *J. Electrochem. Soc.*, 1993, vol. 140:109-111.

G. Gustafsson et. al., Flexible Light-Emitting Diodes Made From Soluble Conducting Polymers, *Nature*, 1992, vol. 357:477-479.

Y. Wang, Photoconductive Materials, *Kirk-Othmer Encyclopedia of Chemical Technology*, Fourth Edition, 1996, vol. 18:837-860.

\* cited by examiner



FIG. 1



FIG. 2

## 1

## ELECTRICALLY CONDUCTIVE POLYMER COMPOSITIONS

## RELATED U.S. APPLICATIONS

This application claims priority to provisional application, Ser. No. 60/694,276, filed Jun. 27, 2005.

## BACKGROUND INFORMATION

## 1. Field of the Disclosure

This disclosure relates generally to electrically conductive polymer compositions, and their use in organic electronic devices.

## 2. Description of the Related Art

Organic electronic devices define a category of products that include an active layer. Such devices convert electrical energy into radiation, detect signals through electronic processes, convert radiation into electrical energy, or include one or more organic semiconductor layers.

Organic light-emitting diodes (OLEDs) are organic electronic devices comprising an organic layer capable of electroluminescence. OLEDs containing conducting polymers can have the following configuration:

anode/buffer layer/EL material/cathode

The anode is typically any material that has the ability to inject holes into the EL material, such as, for example, indium/tin oxide (ITO). The anode is optionally supported on a glass or plastic substrate. EL materials include fluorescent compounds, fluorescent and phosphorescent metal complexes, conjugated polymers, and combinations and mixtures thereof. The cathode is typically any material (such as, e.g., Ca or Ba) that has the ability to inject electrons into the EL material.

The buffer layer is typically an electrically conducting polymer and facilitates the injection of holes from the anode into the EL material layer. Typical conducting polymers employed as buffer layers include polyaniline and polydioxothiophenes such as poly(3,4-ethylenedioxythiophene) (PEDT). These materials can be prepared by polymerizing aniline or dioxythiophene monomers in aqueous solution in the presence of a water soluble polymeric acid, such as poly(styrenesulfonic acid) (PSS), as described in, for example, U.S. Pat. No. 5,300,575.

The aqueous electrically conductive polymer dispersions synthesized with water soluble polymeric sulfonic acids, however, have undesirably low pH levels. The low pH can contribute to decreased stress life of an EL device containing such a buffer layer, and contribute to corrosion within the device. Accordingly, there is a need for compositions and layers prepared therefrom having improved properties.

Electrically conducting polymers having the ability to carry a high current when subjected to a low electrical voltage also have utility as electrodes for electronic devices, such as thin film field effect transistors. In such transistors, an organic semiconducting film which has high mobility for electron and/or hole charge carriers, is present between source and drain electrodes. A gate electrode is on the opposite side of the semiconducting polymer layer. To be useful for the electrode application, the electrically conducting polymers and the liquids for dispersing or dissolving the electrically conducting polymers have to be compatible with the semiconducting polymers and the solvents for the semiconducting polymers to avoid re-dissolution of either conducting polymers or semiconducting polymers. Many conductive polymers have con-

## 2

ductivities which are too low for use as electrodes. Accordingly, there is a need for improved conductive polymers.

Thus, there is a continuing need for electrically conductive polymer compositions having improved chemical, physical and electrical properties.

## SUMMARY

There is provided an electrically conductive polymer composition comprising a first electrically conductive polymer doped with an organic solvent wettable fluorinated acid polymer in admixture with a second electrically conductive polymer doped with an organic solvent non-wettable fluorinated acid polymer.

15 In another embodiment, there is provided an aqueous dispersion of an electrically conductive polymer composition, comprising a first electrically conductive polymer doped with an organic solvent wettable fluorinated acid polymer in admixture with a second electrically conductive polymer 20 doped with an organic solvent non-wettable fluorinated acid polymer.

In another embodiment, electronic devices comprising at least one layer comprising the new conductive polymer composition are provided.

25 The foregoing general description and the following detailed description are exemplary and explanatory only and are not restrictive of the invention, as defined in the appended claims.

## BRIEF DESCRIPTION OF THE DRAWINGS

The invention is illustrated by way of example and not limitation in the accompanying figures.

FIG. 1 is a diagram illustrating contact angle.

35 FIG. 2 is a schematic diagram of an organic electronic device.

40 Skilled artisans appreciate that objects in the figures are illustrated for simplicity and clarity and have not necessarily been drawn to scale. For example, the dimensions of some of the objects in the figures may be magnified relative to other objects to help to improve understanding of embodiments.

## DETAILED DESCRIPTION

45 In one embodiment, there is provided an electrically conductive polymer composition, comprising a first electrically conductive polymer doped with an organic solvent wettable fluorinated acid polymer in admixture with a second electrically conductive polymer doped with an organic solvent non-wettable fluorinated acid polymer.

50 Many aspects and embodiments are described herein and are exemplary and not limiting. After reading this specification, skilled artisans will appreciate that other aspects and embodiments are possible without departing from the scope of the disclosure and appended claims.

55 As used herein, the term "electrically conductive polymer" refers to any polymer or oligomer which is inherently or intrinsically capable of electrical conductivity without the addition of carbon black or conductive metal particles. The 60 term "polymer" encompasses homopolymers and copolymers. The term "electrical conductivity" includes conductive and semi-conductive. In one embodiment, films made from the doped electrically conductive polymer have a conductivity of at least  $10^{-7}$  S/cm. The term "doped" is intended to 65 mean that the electrically conductive polymer has a polymeric counterion derived from a polymeric acid to balance the charge on the conductive polymer. The term "organic

solvent wettable" refers to a material which, when formed into a film, is wettable by organic solvents. The term also includes polymeric acids which are not film-forming alone, but which form an electrically conductive polymer composition which is wettable. In one embodiment, the organic solvent wettable material forms a film which is wettable by phenylhexane with a contact angle less than 40°. The term "organic solvent non-wettable" refers to a material which, when formed into a film, is not wettable by organic solvents. The term also includes polymeric acids that are not film-forming alone, but which form an electrically conductive polymer composition which is non-wettable. In one embodiment, the organic solvent non-wettable material forms a film which on which phenylhexane has a contact angle greater than 40°. The term "fluorinated acid polymer" refers to a polymer having acidic groups, where at least some of the hydrogens have been replaced by fluorine. The term "acidic group" refers to a group capable of ionizing to donate a hydrogen ion to a base to form a salt. The term "in admixture with" is intended to mean that one material is physically mixed with another material. The composition can comprise one or more electrically conductive polymers doped with an organic solvent wettable fluorinated polymeric acid in admixture with one or more electrically conductive polymers doped with an organic solvent non-wettable fluorinated polymeric acid.

### 1. Electrically Conductive Polymers

Any electrically conductive polymer can be used in the new composition. In one embodiment, the electrically conductive polymer will form a film which has a conductivity of at least  $10^{-7}$  S/cm. The conductive polymers suitable for the new composition can be homopolymers, or they can be co-polymers of two or more respective monomers. The monomer from which the conductive polymer is formed, is referred to as a "precursor monomer". A copolymer will have more than one precursor monomer. In its simplest form, a copolymer comprises two monomers, which may have different structural repeat units, or the same structural repeat unit with different substituents on each.

In one embodiment, the first conductive polymer is made from at least one precursor monomer selected from thiophenes, pyrroles, anilines, and polycyclic aromatics. The polymers made from these monomers are referred to herein as polythiophenes, polypyrrroles, polyanilines, and polycyclic aromatic polymers, respectively. The term "polycyclic aromatic" refers to compounds having more than one aromatic ring. The rings may be joined by one or more bonds, or they may be fused together. The term "aromatic ring" is intended to include heteroaromatic rings. A "polycyclic heteroaromatic" compound has at least one heteroaromatic ring.

In one embodiment, thiophene monomers contemplated for use to form the electrically conductive polymer in the new composition comprise Formula I below:



(I)

wherein:

R<sup>1</sup> is independently selected so as to be the same or different at each occurrence and is selected from hydrogen, alkyl, alkenyl, alkoxy, alkanoyl, alkythio, aryloxy, alky-

thioalkyl, alkylaryl, arylalkyl, amino, alkylamino, dialkylamino, aryl, alkylsulfinyl, alkoxyalkyl, alkylsulfonyl, arylthio, arylsulfinyl, alkoxy carbonyl, arylsulfonyl, acrylic acid, phosphoric acid, phosphonic acid, halogen, nitro, cyano, hydroxyl, epoxy, silane, siloxane, alcohol, benzyl, carboxylate, ether, ether carboxylate, amidosulfonate, ether sulfonate, ester sulfonate, and urethane; or both R<sup>1</sup> groups together may form an alkylene or alkenylene chain completing a 3, 4, 5, 6, or 7-membered aromatic or alicyclic ring, which ring may optionally include one or more divalent nitrogen, sulfur or oxygen atoms.

As used herein, the term "alkyl" refers to a group derived from an aliphatic hydrocarbon and includes linear, branched and cyclic groups which may be unsubstituted or substituted. The term "heteroalkyl" is intended to mean an alkyl group, wherein one or more of the carbon atoms within the alkyl group has been replaced by another atom, such as nitrogen, oxygen, sulfur, and the like. The term "alkylene" refers to an alkyl group having two points of attachment.

As used herein, the term "alkenyl" refers to a group derived from an aliphatic hydrocarbon having at least one carbon-carbon double bond, and includes linear, branched and cyclic groups which may be unsubstituted or substituted. The term "heteroalkenyl" is intended to mean an alkenyl group, wherein one or more of the carbon atoms within the alkenyl group has been replaced by another atom, such as nitrogen, oxygen, sulfur, and the like. The term "alkenylene" refers to an alkenyl group having two points of attachment.

As used herein, the following terms for substituent groups refer to the formulae given below:

- "alcohol" —R<sup>3</sup>—OH
- "amido" —R<sup>3</sup>—C(O)N(R<sup>6</sup>)R<sup>6</sup>
- "amidosulfonate" —R<sup>3</sup>—C(O)N(R<sup>6</sup>)R<sup>4</sup>—SO<sub>3</sub>Z
- "benzyl" —CH<sub>2</sub>—C<sub>6</sub>H<sub>5</sub>
- "carboxylate" —R<sup>3</sup>—C(O)O—Z or —R<sup>3</sup>—O—C(O)—Z
- "ether" —R<sup>3</sup>—(O—R<sup>5</sup>)<sub>p</sub>—O—R<sup>5</sup>
- "ether carboxylate" —R<sup>3</sup>—O—R<sup>4</sup>—C(O)O—Z or —R<sup>3</sup>—O—R<sup>4</sup>—O—C(O)—Z
- "ether sulfonate" —R<sup>3</sup>—O—R<sup>4</sup>—SO<sub>3</sub>Z
- "ester sulfonate" —R<sup>3</sup>—O—C(O)—R<sup>4</sup>—SO<sub>3</sub>Z
- "sulfoniimide" —R<sup>3</sup>—SO<sub>2</sub>—NH—SO<sub>2</sub>—R<sup>5</sup>
- "urethane" —R<sup>3</sup>—O—C(O)—N(R<sup>6</sup>)<sub>2</sub>

where all "R" groups are the same or different at each occurrence and:

R<sup>3</sup> is a single bond or an alkylene group

R<sup>4</sup> is an alkylene group

R<sup>5</sup> is an alkyl group

R<sup>6</sup> is hydrogen or an alkyl group

p is 0 or an integer from 1 to 20

Z is H, alkali metal, alkaline earth metal, N(R<sup>5</sup>)<sub>4</sub> or R<sup>5</sup>

Any of the above groups may further be unsubstituted or substituted, and any group may have F substituted for one or more hydrogens, including perfluorinated groups. In one embodiment, the alkyl and alkylene groups have from 1-20 carbon atoms.

In one embodiment, in the thiophene monomer, both R<sup>1</sup> together form —O—(CHY)<sub>m</sub>—O—, where m is 2 or 3, and Y is the same or different at each occurrence and is selected from hydrogen, halogen, alkyl, alcohol, amidosulfonate, benzyl, carboxylate, ether, ether carboxylate, ether sulfonate, ester sulfonate, and urethane, where the Y groups may be partially or fully fluorinated. In one embodiment, all Y are hydrogen. In one embodiment, the polythiophene is poly(3, 4-ethylenedioxythiophene). In one embodiment, at least one Y group is not hydrogen. In one embodiment, at least one Y group is a substituent having F substituted for at least one hydrogen. In one embodiment, at least one Y group is perfluorinated.

In one embodiment, the thiophene monomer has Formula I(a):



(Ia)

wherein:

R<sup>7</sup> is the same or different at each occurrence and is selected from hydrogen, alkyl, heteroalkyl, alkenyl, heteroalkenyl, alcohol, amidosulfonate, benzyl, carboxylate, ether, ether carboxylate, ether sulfonate, ester sulfonate, and urethane, with the proviso that at least one R<sup>7</sup> is not hydrogen, and

m is 2 or 3.

In one embodiment of Formula I(a), m is two, one R<sup>7</sup> is an alkyl group of more than 5 carbon atoms, and all other R<sup>7</sup> are hydrogen. In one embodiment of Formula I(a), at least one R<sup>7</sup> group is fluorinated. In one embodiment, at least one R<sup>7</sup> group has at least one fluorine substituent. In one embodiment, the R<sup>7</sup> group is fully fluorinated.

In one embodiment of Formula I(a), the R<sup>7</sup> substituents on the fused alicyclic ring on the thiophene offer improved solubility of the monomers in water and facilitate polymerization in the presence of the fluorinated acid polymer.

In one embodiment of Formula I(a), m is 2, one R<sup>7</sup> is sulfonic acid-propylene-ether-methylene and all other R<sup>7</sup> are hydrogen. In one embodiment, m is 2, one R<sup>7</sup> is propyl-ether-ethylene and all other R<sup>7</sup> are hydrogen. In one embodiment, m is 2, one R<sup>7</sup> is methoxy and all other R<sup>7</sup> are hydrogen. In one embodiment, one R<sup>7</sup> is sulfonic acid difluoromethylene ester methylene (—CH<sub>2</sub>—O—C(O)—CF<sub>2</sub>—SO<sub>3</sub>H), and all other R<sup>7</sup> are hydrogen.

In one embodiment, pyrrole monomers contemplated for use to form the electrically conductive polymer in the new composition comprise Formula II below.



(II)

where in Formula II:

R<sup>1</sup> is independently selected so as to be the same or different at each occurrence and is selected from hydrogen, alkyl, alkenyl, alkoxy, alkanoyl, alkylthio, aryloxy, alkylthioalkyl, alkylaryl, arylalkyl, amino, alkylamino, dialkylamino, aryl, alkylsulfinyl, alkoxyalkyl, alkylsulfonyl, arylthio, arylsulfinyl, alkoxy carbonyl, arylsulfonyl, acrylic acid, phosphoric acid, phosphonic acid, halogen, nitro, cyano, hydroxyl, epoxy, silane, siloxane, alcohol, benzyl, carboxylate, ether, amidosulfonate, ether carboxylate, ether sulfonate, ester sulfonate, and urethane; or both R<sup>1</sup> groups together may form an alkylene or alkenylene chain completing a 3, 4, 5, 6, or 7-membered aromatic or alicyclic ring, which ring may optionally include one or more divalent nitrogen, sulfur or oxygen atoms; and

R<sup>2</sup> is independently selected so as to be the same or different at each occurrence and is selected from hydrogen, alkyl, alkenyl, aryl, alkanoyl, alkylthioalkyl, alkylaryl, arylalkyl, amino, epoxy, silane, siloxane, alcohol, benzyl, carboxylate, ether, ether carboxylate, ether sulfonate, ester sulfonate, and urethane.

In one embodiment, R<sup>1</sup> is the same or different at each occurrence and is independently selected from hydrogen, alkyl, alkenyl, alkoxy, cycloalkyl, cycloalkenyl, alcohol, benzyl, carboxylate, ether, amidosulfonate, ether carboxylate, ether sulfonate, ester sulfonate, urethane, epoxy, silane, siloxane, and alkyl substituted with one or more of sulfonic acid, carboxylic acid, acrylic acid, phosphoric acid, phosphonic acid, halogen, nitro, cyano, hydroxyl, epoxy, silane, or siloxane moieties.

In one embodiment, R<sup>2</sup> is selected from hydrogen, alkyl, and alkyl substituted with one or more of sulfonic acid, carboxylic acid, acrylic acid, phosphoric acid, phosphonic acid, halogen, cyano, hydroxyl, epoxy, silane, or siloxane moieties.

In one embodiment, the pyrrole monomer is unsubstituted and both R<sup>1</sup> and R<sup>2</sup> are hydrogen.

In one embodiment, both R<sup>1</sup> together form a 6- or 7-membered alicyclic ring, which is further substituted with a group selected from alkyl, heteroalkyl, alcohol, benzyl, carboxylate, ether, ether carboxylate, ether sulfonate, ester sulfonate, and urethane. These groups can improve the solubility of the monomer and the resulting polymer. In one embodiment, both R<sup>1</sup> together form a 6- or 7-membered alicyclic ring, which is further substituted with an alkyl group. In one embodiment, both R<sup>1</sup> together form a 6- or 7-membered alicyclic ring, which is further substituted with an alkyl group having at least 1 carbon atom.

In one embodiment, both R<sup>1</sup> together form —O—(CHY)<sub>m</sub>—O—, where m is 2 or 3, and Y is the same or different at each occurrence and is selected from hydrogen, alkyl, alcohol, benzyl, carboxylate, amidosulfonate, ether, ether carboxylate, ether sulfonate, ester sulfonate, and urethane. In one embodiment, at least one Y group is not hydrogen. In one embodiment, at least one Y group is a substituent having F substituted for at least one hydrogen. In one embodiment, at least one Y group is perfluorinated.

In one embodiment, aniline monomers contemplated for use to form the electrically conductive polymer in the new composition comprise Formula III below.



wherein:

a is 0 or an integer from 1 to 4;

b is an integer from 1 to 5, with the proviso that a+b=5; and

R<sup>1</sup> is independently selected so as to be the same or different at each occurrence and is selected from hydrogen, alkyl, alkenyl, alkoxy, alkanoyl, alkylthio, aryloxy, alkylthioalkyl, alkylaryl, arylalkyl, amino, alkylamino, dialkylamino, aryl, alkylsulfinyl, alkoxyalkyl, alkylsulfonyl, arylthio, arylsulfinyl, arylsulfonyl, acrylic acid, phosphoric acid, phosphonic acid, halogen, nitro, cyano, hydroxyl, epoxy, silane, siloxane, alcohol, benzyl, carboxylate, ether, ether carboxylate, amidosulfonate, ether sulfonate, ester sulfonate, and urethane; or both R<sup>1</sup> groups together may form an alkylene or alkenylene chain completing a 3, 4, 5, 6, or 7-membered aromatic or alicyclic ring, which ring may optionally include one or more divalent nitrogen, sulfur or oxygen atoms.

When polymerized, the aniline monomeric unit can have Formula IV(a) or Formula IV(b) shown below, or a combination of both formulae.

10

5

15

20

25

30

35

IV(a)



40

IV(b)



45

50

55

60

where a, b and R<sup>1</sup> are as defined above.

In one embodiment, the aniline monomer is unsubstituted and a=0.

In one embodiment, a is not 0 and at least one R<sup>1</sup> is fluorinated. In one embodiment, at least one R<sup>1</sup> is perfluorinated.

In one embodiment, fused polycyclic heteroaromatic monomers contemplated for use to form the electrically conductive polymer in the new composition have two or more fused aromatic rings, at least one of which is heteroaromatic. In one embodiment, the fused polycyclic heteroaromatic monomer has Formula V:



(V)

wherein:

Q is S or NR<sup>6</sup>;

R<sup>6</sup> is hydrogen or alkyl;

R<sup>8</sup>, R<sup>9</sup>, R<sup>10</sup>, and R<sup>11</sup> are independently selected so as to be the same or different at each occurrence and are selected from hydrogen, alkyl, alkenyl, alkoxy, alkanoyl, alkylthio, aryloxy, alkylthioalkyl, alkylaryl, arylalkyl, amino, alkylamino, dialkylamino, aryl, alkylsulfinyl, alkoxyalkyl, alkylsulfonyl, arylthio, arylsulfinyl, arylsulfonyl, acrylic acid, phosphoric acid, phosphonic acid, halogen, nitro, cyano, hydroxyl, epoxy, silane, siloxane, alcohol, benzyl, carboxylate, ether, ether carboxylate, amidosulfonate, ether sulfonate, ester sulfonate, and urethane; and

at least one of R<sup>8</sup> and R<sup>9</sup>, R<sup>9</sup> and R<sup>10</sup>, and R<sup>10</sup> and R<sup>11</sup> together form an alkenylene chain completing a 5 or 6-membered aromatic ring, which ring may optionally include one or more divalent nitrogen, sulfur or oxygen atoms.

In one embodiment, the fused polycyclic heteroaromatic monomer has Formula V(a), V(b), V(c), V(d), V(e), V(f), and V(g):

(Va)



(Vb)



(Vc)



-continued



wherein:

Q is S or NH; and

T is the same or different at each occurrence and is selected from S, NR<sup>6</sup>, O, SiR<sup>6</sup><sub>2</sub>, Se, and PR<sup>6</sup>;R<sup>6</sup> is hydrogen or alkyl.

The fused polycyclic heteroaromatic monomers may be further substituted with groups selected from alkyl, heteroalkyl, alcohol, benzyl, carboxylate, ether, ether carboxylate, ether sulfonate, ester sulfonate, and urethane. In one embodiment, the substituent groups are fluorinated. In one embodiment, the substituent groups are fully fluorinated.

In one embodiment, the fused polycyclic heteroaromatic monomer is a thieno(thiophene). Such compounds have been discussed in, for example, *Macromolecules*, 34, 5746-5747 (2001); and *Macromolecules*, 35, 7281-7286 (2002). In one embodiment, the thieno(thiophene) is selected from thieno(2,3-b)thiophene, thieno(3,2-b)thiophene, and thieno(3,4-b)thiophene. In one embodiment, the thieno(thiophene) monomer is substituted with at least one group selected from alkyl, heteroalkyl, alcohol, benzyl, carboxylate, ether, ether carboxylate, ether sulfonate, ester sulfonate, and urethane. In one embodiment, the substituent groups are fluorinated. In one embodiment, the substituent groups are fully fluorinated.

In one embodiment, polycyclic heteroaromatic monomers contemplated for use to form the copolymer in the new composition comprise Formula VI:



wherein:

Q is S or NR<sup>6</sup>;T is selected from S, NR<sup>6</sup>, O, SiR<sup>6</sup><sub>2</sub>, Se, and PR<sup>6</sup>;

E is selected from alkenylene, arylene, and heteroarylene;

R<sup>6</sup> is hydrogen or alkyl;

R<sup>12</sup> is the same or different at each occurrence and is selected from hydrogen, alkyl, alkenyl, alkoxy, alkanoyl, alkylthio, aryloxy, alkylthioalkyl, alkylaryl, arylalkyl, amino, alkylamino, dialkylamino, aryl, alkylsulfinyl, alkoxyalkyl, alkylsulfonyl, arylthio, arylsulfinyl, alkoxy carbonyl, arylsulfonyl, acrylic acid, phosphoric acid, phosphonic acid, halogen, nitro, nitrile, cyano, hydroxyl, epoxy, silane, siloxane, alcohol, benzyl, carboxylate, ether, ether carboxylate, amidosulfonate, ether sulfonate, ester sulfonate, and urethane; or both R<sup>12</sup> groups together may form an alkylene or alkenylene chain completing a 3, 4, 5, 6, or 7-membered aromatic or alicyclic ring, which ring may optionally include one or more divalent nitrogen, sulfur or oxygen atoms.

In one embodiment, the electrically conductive polymer is a copolymer of a precursor monomer and at least one second monomer. Any type of second monomer can be used, so long as it does not detrimentally affect the desired properties of the

copolymer. In one embodiment, the second monomer comprises no more than 50% of the copolymer, based on the total number of monomer units. In one embodiment, the second monomer comprises no more than 30%, based on the total number of monomer units. In one embodiment, the second monomer comprises no more than 10%, based on the total number of monomer units.

Exemplary types of monomers comprising the second conductive polymer include, but are not limited to, alkenyl, alkynyl, arylene, and heteroarylene. Examples of second monomers include, but are not limited to, fluorene, oxadiazole, thiadiazole, benzothiadiazole, phenylenevinylene, phenyleneethynylene, pyridine, diazines, and triazines, all of which may be further substituted.

In one embodiment, the copolymers are made by first forming an intermediate precursor monomer having the structure A-B-C, where A and C represent first precursor monomers, which can be the same or different, and B represents a second precursor monomer. The A-B-C intermediate precursor monomer can be prepared using standard synthetic organic techniques, such as Yamamoto, Stille, Grignard metathesis, Suzuki, and Negishi couplings. The copolymer is then formed by oxidative polymerization of the intermediate precursor monomer alone, or with one or more additional precursor monomers.

In one embodiment, the electrically conductive polymer is a copolymer of two or more precursor monomers. In one embodiment, the first precursor monomers are selected from a thiophene, a pyrrole, an aniline, and a polycyclic aromatic.

## 50 2. Organic Solvent Wettable Fluorinated Acid Polymer

The organic solvent wettable fluorinated acid polymer (hereinafter referred to as a "wettable FAP") can be any polymer which is fluorinated, has acidic groups, and is wettable by organic solvents. As used herein, the term "fluorinated" means that at least one hydrogen bonded to a carbon has been replaced with a fluorine. The term includes partially and fully fluorinated materials. In one embodiment, the fluorinated acid polymer is highly fluorinated. The term "highly fluorinated" means that at least 50% of the available hydrogens bonded to a carbon, have been replaced with fluorine. The acidic groups supply an ionizable proton. In one embodiment, the acidic group has a pKa of less than 3. In one embodiment, the acidic group has a pKa of less than 0. In one embodiment, the acidic group has a pKa of less than -5. The acidic group can be attached directly to the polymer backbone, or it can be attached to side chains on the polymer backbone. Examples of acidic groups include, but are not

## 11

limited to, carboxylic acid groups, sulfonic acid groups, sulfonimide groups, phosphoric acid groups, phosphonic acid groups, and combinations thereof. The acidic groups can all be the same, or the polymer may have more than one type of acidic group.

In one embodiment, the wettable FAP forms a film which is wettable by phenylhexane. In one embodiment, phenylhexane forms drops having a contact angle no greater than 40°. As used herein, the term "contact angle" is intended to mean the angle  $\phi$  shown in FIG. 1. For a droplet of liquid medium, angle  $\phi$  is defined by the intersection of the plane of the surface and a line from the outer edge of the droplet to the surface. Furthermore, angle  $\phi$  is measured after the droplet has reached an equilibrium position on the surface after being applied, i.e., "static contact angle". The film of the organic solvent wettable fluorinated polymeric acid is represented as the surface. In one embodiment, the contact angle is no greater than 35°. In one embodiment, the contact angle is no greater than 30°. The methods for measuring contact angles are well known.

In one embodiment, the wettable FAP is water-soluble. In one embodiment, the wettable FAP is dispersible in water.

In one embodiment, the polymer backbone is fluorinated. Examples of suitable polymeric backbones include, but are not limited to, polyolefins, polyacrylates, polymethacrylates, polyimides, polyamides, polyaramids, polyacrylamides, polystyrenes, and copolymers thereof. In one embodiment, the polymer backbone is highly fluorinated. In one embodiment, the polymer backbone is fully fluorinated.

In one embodiment, the acidic groups are selected from sulfonic acid groups and sulfonimide groups. In one embodiment, the acidic groups are on a fluorinated side chain. In one embodiment, the fluorinated side chains are selected from alkyl groups, alkoxy groups, amido groups, ether groups, and combinations thereof.

In one embodiment, the wettable FAP has a fluorinated olefin backbone, with pendant fluorinated ether sulfonate, fluorinated ester sulfonate, or fluorinated ether sulfonimide groups. In one embodiment, the polymer is a copolymer of 1,1-difluoroethylene and 2-(1,1-difluoro-2-(trifluoromethyl)allyloxy)-1,1,2,2-tetrafluoroethanesulfonic acid. In one embodiment, the polymer is a copolymer of ethylene and 2-(2-(1,2,2-trifluorovinylxy)-1,1,2,3,3-hexafluoropropoxy)-1,1,2,2-tetrafluoroethanesulfonic acid. These copolymers can be made as the corresponding sulfonyl fluoride polymer and then can be converted to the sulfonic acid form.

In one embodiment, the wettable FAP is homopolymer or copolymer of a fluorinated and partially sulfonated poly(arylene ether sulfone). The copolymer can be a block copolymer. Examples of comonomers include, but are not limited to butadiene, butylene, isobutylene, styrene, and combinations thereof.

In one embodiment, the wettable FAP is a homopolymer or copolymer of monomers having Formula VII:

(VII)



## 12

where:

b is an integer from 1 to 5,

R<sup>13</sup> is OH or NHR<sup>14</sup>, and

R<sup>14</sup> is alkyl, fluoroalkyl, sulfonylalkyl, or sulfonylfluoroalkyl.

In one embodiment, the monomer is "SFS" or SFSI" shown below:

10



20

SFS

SFSI

After polymerization, the polymer can be converted to the acid form.

In one embodiment, the wettable FAP is a homopolymer or copolymer of a trifluorostyrene having acidic groups. In one embodiment, the trifluorostyrene monomer has Formula VIII:

30



(VIII)

where:

W is selected from (CF<sub>2</sub>)<sub>q</sub>, O(CF<sub>2</sub>)<sub>q</sub>, S(CF<sub>2</sub>)<sub>q</sub>, (CF<sub>2</sub>)<sub>q</sub>O(CF<sub>2</sub>)<sub>q</sub>, and SO<sub>2</sub>(CF<sub>2</sub>)<sub>q</sub>,

b is independently an integer from 1 to 5,

R<sup>13</sup> is OH or NHR<sup>14</sup>, and

R<sup>14</sup> is alkyl, fluoroalkyl, sulfonylalkyl, or sulfonylfluoroalkyl.

50

In one embodiment, the monomer containing W equal to S(CF<sub>2</sub>)<sub>q</sub> is polymerized then oxidized to give the polymer containing W equal to SO<sub>2</sub>(CF<sub>2</sub>)<sub>q</sub>. In one embodiment, the polymer containing R<sup>13</sup> equal to F is converted its acid form where R<sup>13</sup> is equal to OH or NHR<sup>14</sup>.

55

In one embodiment, the wettable FAP is a sulfonimide polymer having Formula IX:

60



(IX)

where:

R<sub>f</sub> is selected from fluorinated alkylene, fluorinated heteroalkylene, fluorinated arylene, or fluorinated heteroarylene;

## 13

$R_g$  is selected from fluorinated alkylene, fluorinated heteroalkylene, fluorinated arylene, fluorinated heteroarylene, arylene, or heteroarylene; and n is at least 4.

In one embodiment of Formula IX,  $R_f$  and  $R_g$  are perfluoroalkylene groups. In one embodiment,  $R_f$  and  $R_g$  are perfluorobutylene groups. In one embodiment,  $R_f$  and  $R_g$  contain ether oxygens. In one embodiment, n is greater than 20.

In one embodiment, the wettable FAP comprises a fluorinated polymer backbone and a side chain having Formula X:



where:

$R_g$  is selected from fluorinated alkylene, fluorinated heteroalkylene, fluorinated arylene, fluorinated heteroarylene, arylene, or heteroarylene;

$R^{15}$  is a fluorinated alkylene group or a fluorinated heteroalkylene group;

$R^{16}$  is a fluorinated alkyl or a fluorinated aryl group; and a is 0 or an integer from 1 to 4.

In one embodiment, the wettable FAP has Formula XI:



where:

$R^{16}$  is a fluorinated alkyl or a fluorinated aryl group; a, b, c, d, and e are each independently 0 or an integer from 1 to 4; and n is at least 4.

The synthesis of these fluorinated acid polymers has been described in, for example, A. Feiring et al., J. Fluorine Chemistry 2000, 105, 129-135; A. Feiring et al., Macromolecules 2000, 33, 9262-9271; D. D. Desmarteau, J. Fluorine Chem. 1995, 72, 203-208; A. J. Appleby et al., J. Electrochem. Soc. 1993, 140(1), 109-111; and Desmarteau, U.S. Pat. No. 5,463, 005.

In one embodiment, the wettable FAP comprises at least one repeat unit derived from an ethylenically unsaturated compound having the Formula XII:



wherein d is 0, 1, or 2;

$R^{17}$  to  $R^{20}$  are independently H, halogen, alkyl or alkoxy of 1 to 10 carbon atoms, Y,  $C(R_f)(R_g)OR^{21}$ ,  $R^4Y$  or  $OR^4Y$ ;

## 14

$Y$  is  $\text{COE}^2$ ,  $\text{SO}_2\text{E}^2$ , or sulfonimide;

$R^{21}$  is hydrogen or an acid-labile protecting group;

$R_f$  is the same or different at each occurrence and is a fluoroalkyl group of 1 to 10 carbon atoms, or taken together are  $(\text{CF}_2)_e$  where e is 2 to 10;

$R^4$  is an alkylene group;

$E^2$  is OH, halogen, or  $\text{OR}^7$ ; and

$R^5$  is an alkyl group;

with the proviso that at least one of  $R^{17}$  to  $R^{20}$  is  $Y$ ,  $R^4Y$  or  $OR^4Y$ .

$R^4$ ,  $R^5$ , and  $R^{17}$  to  $R^{20}$  may optionally be substituted by halogen or ether oxygen.

Some illustrative, but nonlimiting, examples of representative monomers of Formula XII, in which d=0, are presented in Formulas XIIa-XIId, below:



(XIIa)

(XI)

-continued



(XIIb)



(XIIc)



(XIId)

60 wherein  $R^{21}$  is a group capable of forming or rearranging to a tertiary cation, more typically an alkyl group of 1 to 20 carbon atoms, and most typically t-butyl.

Compounds of structure (XII) wherein d=0, (e.g., Formula XII-a), may be prepared by cycloaddition reaction of unsaturated compounds of structure (XIII) with quadricyclane (tetraacyclo[2.2.1.0<sup>2,6</sup>0<sup>3,5</sup>]heptane) as shown in the equation below.



The reaction may be conducted at temperatures ranging from about 0° C. to about 200° C., more typically from about 30° C. to about 150° C. in the absence or presence of an inert solvent such as diethyl ether. For reactions conducted at or above the boiling point of one or more of the reagents or solvent, a closed reactor is typically used to avoid loss of volatile components. Compounds of structure (XII) with higher values of d (i.e., d=1 or 2) may be prepared by reaction of compounds of structure (XII) with d=0 with cyclopentadiene, as is known in the art.

In one embodiment, the wettable FAP is a copolymer which also comprises a repeat unit derived from at least one fluoroolefin, which is an ethylenically unsaturated compound containing at least one fluorine atom attached to an ethylenically unsaturated carbon. The fluoroolefin comprises 2 to 20 carbon atoms. Representative fluoroolefins include, but are not limited to, tetrafluoroethylene, hexafluoropropylene, chlorotrifluoroethylene, vinylidene fluoride, vinyl fluoride, perfluoro-(2,2-dimethyl-1,3-dioxole), perfluoro-(2-methylene-4-methyl-1,3-dioxolane),  $\text{CF}_2=\text{CFO}(\text{CF}_2)_t\text{CF}=\text{CF}_2$ , where t is 1 or 2, and R<sub>f</sub>"OCF=CF<sub>2</sub> wherein R<sub>f</sub>" is a saturated fluoroalkyl group of from 1 to about ten carbon atoms. In one embodiment, the comonomer is tetrafluoroethylene.

**3. Organic Solvent Non-Wettable Fluorinated Acid Polymer**  
The organic solvent non-wettable fluorinated acid polymer (hereinafter referred to as a “non-wettable FAP”) can be any polymer which is fluorinated, has acidic groups, and is not wettable by organic solvents. In one embodiment, the acidic group has a pKa of at less than 3. In one embodiment, the acidic group has a pKa of less than 0. In one embodiment, the acidic group has a pKa of less than -5. The acidic groups can be attached directly to the polymer backbone, or they can be attached to side chains on the polymer backbone. Examples of acidic groups include, but are not limited to, carboxylic acid groups, sulfonic acid groups, sulfonimide groups, phosphoric acid groups, phosphonic acid groups, and combinations thereof. The acidic groups can all be the same, or the polymer may have more than one type of acidic group.

In one embodiment, the non-wettable FAP forms a film that is not wettable by phenylhexane. In one embodiment, phenylhexane forms drops having a contact angle greater than 40°. In one embodiment, the contact angle is greater than 45°. In one embodiment, the contact angle is greater than 50°.

In one embodiment, the fluorinated acid polymer comprises a polymeric backbone having pendant groups comprising siloxane sulfonic acid. In one embodiment, the siloxane pendant groups have the formula below:



wherein:

a is from 1 to b;

b is from 1 to 3;

R<sup>22</sup> is a non-hydrolyzable group independently selected from the group consisting of alkyl, aryl, and arylalkyl;

R<sup>23</sup> is a bidentate alkylene radical, which may be substituted by one or more ether oxygen atoms, with the proviso that R<sup>23</sup> has at least two carbon atoms linearly disposed between Si and R<sub>j</sub>; and

5 R<sub>j</sub> is a perfluoralkylene radical, which may be substituted by one or more ether oxygen atoms.

In one embodiment, the fluorinated acid polymer having pendant siloxane groups has a fluorinated backbone. In one embodiment, the backbone is perfluorinated.

10 In one embodiment, the fluorinated acid polymer has a fluorinated backbone and pendant groups represented by the Formula (XIV)



wherein R<sub>f</sub><sup>2</sup> is F or a perfluoroalkyl radical having 1-10 carbon atoms either unsubstituted or substituted by one or more ether oxygen atoms, h=0 or 1, i=0 to 3, and g=0 or 1.

20 In one embodiment, the fluorinated acid polymer has formula (XV)



where j≥0, k≥0 and 4≤(j+k)≤199, Q<sup>1</sup> and Q<sup>2</sup> are F or H, R<sub>f</sub><sup>2</sup> is F or a perfluoroalkyl radical having 1-10 carbon atoms either unsubstituted or substituted by one or more ether oxygen atoms, h=0 or 1, i=0 to 3, g=0 or 1, and E<sup>4</sup> is H or an alkali metal. In one embodiment R<sub>f</sub><sup>2</sup> is —CF<sub>3</sub>, g=1, h=1, and i=1. In one embodiment the pendant group is present at a concentration of 3-10 mol-%.

35 40 In one embodiment, Q<sup>1</sup> is H, k≥0, and Q<sup>2</sup> is F, which may be synthesized according to the teachings of Connolly et al., U.S. Pat. No. 3,282,875. In another preferred embodiment, Q<sup>1</sup> is H, Q<sup>2</sup> is H, g=0, R<sub>f</sub><sup>2</sup> is F, h=1, and i=1, which may be synthesized according to the teachings of co-pending application Ser. No. 60/105,662. Still other embodiments may be synthesized according to the various teachings in Drysdale et al., WO 9831716(A1), and co-pending US applications Choi et al., WO 99/52954(A1), and 60/176,881.

45 In one embodiment, the non-wettable FAP is a colloid-forming polymeric acid. As used herein, the term “colloid-forming” refers to materials that are insoluble in water, and form colloids when dispersed into an aqueous medium. The colloid-forming polymeric acids typically have a molecular weight in the range of about 10,000 to about 4,000,000. In one embodiment, the polymeric acids have a molecular weight of about 100,000 to about 2,000,000. Colloid particle size typically ranges from 2 nanometers (nm) to about 140 nm. In one embodiment, the colloids have a particle size of 2 nm to about 30 nm. Any colloid-forming polymeric material having acidic

55 60 protons can be used. In one embodiment, the colloid-forming fluorinated polymeric acid has acidic groups selected from carboxylic groups, sulfonic acid groups, and sulfonimide groups. In one embodiment, the colloid-forming fluorinated polymeric acid is a polymeric sulfonic acid. In one embodiment, the colloid-forming polymeric sulfonic acid is perfluorinated. In one embodiment, the colloid-forming polymeric sulfonic acid is a perfluoroalkylenesulfonic acid.

In one embodiment, the non-wettable colloid-forming FAP is a highly-fluorinated sulfonic acid polymer ("FSA polymer"). "Highly fluorinated" means that at least about 50% of the total number of halogen and hydrogen atoms in the polymer are fluorine atoms, an in one embodiment at least about 75%, and in another embodiment at least about 90%. In one embodiment, the polymer is perfluorinated. The term "sulfonate functional group" refers to either to sulfonic acid groups or salts of sulfonic acid groups, and in one embodiment alkali metal or ammonium salts. The functional group is represented by the formula  $—SO_3E^5$  where  $E^5$  is a cation, also known as a "counterion".  $E^5$  may be H, Li, Na, K or  $N(R_1)(R_2)(R_3)(R_4)$ , and  $R_1, R_2, R_3$ , and  $R_4$  are the same or different and are and in one embodiment H,  $CH_3$  or  $C_2H_5$ . In another embodiment,  $E^5$  is H, in which case the polymer is said to be in the "acid form".  $E^5$  may also be multivalent, as represented by such ions as  $Ca^{++}$ , and  $Al^{+++}$ . It is clear to the skilled artisan that in the case of multivalent counterions, represented generally as  $M^{x+}$ , the number of sulfonate functional groups per counterion will be equal to the valence "x".

In one embodiment, the FSA polymer comprises a polymer backbone with recurring side chains attached to the backbone, the side chains carrying cation exchange groups. Polymers include homopolymers or copolymers of two or more monomers. Copolymers are typically formed from a non-functional monomer and a second monomer carrying the cation exchange group or its precursor, e.g., a sulfonyl fluoride group ( $—SO_2F$ ), which can be subsequently hydrolyzed to a sulfonate functional group. For example, copolymers of a first fluorinated vinyl monomer together with a second fluorinated vinyl monomer having a sulfonyl fluoride group ( $—SO_2F$ ) can be used. Possible first monomers include tetrafluoroethylene (TFE), hexafluoropropylene, vinyl fluoride, vinylidene fluoride, trifluoroethylene, chlorotrifluoroethylene, perfluoro(alkyl vinyl ether), and combinations thereof. TFE is a preferred first monomer.

In other embodiments, possible second monomers include fluorinated vinyl ethers with sulfonate functional groups or precursor groups which can provide the desired side chain in the polymer. Additional monomers, including ethylene, propylene, and  $R—CH=CH_2$  where R is a perfluorinated alkyl group of 1 to 10 carbon atoms, can be incorporated into these polymers if desired. The polymers may be of the type referred to herein as random copolymers, that is, copolymers made by polymerization in which the relative concentrations of the comonomers are kept as constant as possible, so that the distribution of the monomer units along the polymer chain is in accordance with their relative concentrations and relative reactivities. Less random copolymers, made by varying relative concentrations of monomers in the course of the polymerization, may also be used. Polymers of the type called block copolymers, such as those disclosed in European Patent Application No. 1 026 152 A1, may also be used.

In one embodiment, FSA polymers for use in the present invention include a highly fluorinated, and in one embodiment perfluorinated, carbon backbone and side chains represented by the formula



wherein  $R_f^3$  and  $R_f^4$  are independently selected from F, Cl or a perfluorinated alkyl group having 1 to 10 carbon atoms,  $a=0$ , 1 or 2, and  $E^5$  is H, Li, Na, K or  $N(R_1)(R_2)(R_3)(R_4)$  and  $R_1, R_2, R_3$ , and  $R_4$  are the same or different and are and in one embodiment H,  $CH_3$  or  $C_2H_5$ . In another embodiment  $E^5$  is H. As stated above,  $E^5$  may also be multivalent.

In one embodiment, the FSA polymers include, for example, polymers disclosed in U.S. Pat. No. 3,282,875 and in U.S. Pat. Nos. 4,358,545 and 4,940,525. An example of preferred FSA polymer comprises a perfluorocarbon backbone and the side chain represented by the formula



where X is as defined above. FSA polymers of this type are disclosed in U.S. Pat. No. 3,282,875 and can be made by copolymerization of tetrafluoroethylene (TFE) and the perfluorinated vinyl ether  $CF_2=CF—O—CF_2CF(CF_3)—O—CF_2CF_2SO_2F$ , perfluoro(3,6-dioxa-4-methyl-7-octenesulfonyl fluoride) (PDMOF), followed by conversion to sulfonate groups by hydrolysis of the sulfonyl fluoride groups and ion exchanged as necessary to convert them to the desired ionic form. An example of a polymer of the type disclosed in U.S. Pat. Nos. 4,358,545 and 4,940,525 has the side chain  $—O—CF_2CF_2SO_3E^5$ , wherein  $E^5$  is as defined above. This polymer can be made by copolymerization of tetrafluoroethylene (TFE) and the perfluorinated vinyl ether  $CF_2=CF—O—CF_2CF_2SO_2F$ , perfluoro(3-oxa-4-pentenesulfonyl fluoride) (POPF), followed by hydrolysis and further ion exchange as necessary.

In one embodiment, the FSA polymers for use in this invention typically have an ion exchange ratio of less than about 33. In this application, "ion exchange ratio" or "IXR" is defined as number of carbon atoms in the polymer backbone in relation to the cation exchange groups. Within the range of less than about 33, IXR can be varied as desired for the particular application. In one embodiment, the IXR is about 3 to about 33, and in another embodiment about 8 to about 23.

The cation exchange capacity of a polymer is often expressed in terms of equivalent weight (EW). For the purposes of this application, equivalent weight (EW) is defined to be the weight of the polymer in acid form required to neutralize one equivalent of sodium hydroxide. In the case of a sulfonate polymer where the polymer has a perfluorocarbon backbone and the side chain is  $—O—CF_2—CF(CF_3)—O—CF_2—CF_2—SO_3H$  (or a salt thereof), the equivalent weight range which corresponds to an IXR of about 8 to about 23 is about 750 EW to about 1500 EW. IXR for this polymer can be related to equivalent weight using the formula:  $50 IXR + 344 = EW$ . While the same IXR range is used for sulfonate polymers disclosed in U.S. Pat. Nos. 4,358,545 and 4,940,525, e.g., the polymer having the side chain  $—O—CF_2CF_2SO_3H$  (or a salt thereof), the equivalent weight is somewhat lower because of the lower molecular weight of the monomer unit containing a cation exchange group. For the preferred IXR range of about 8 to about 23, the corresponding equivalent weight range is about 575 EW to about 1325 EW. IXR for this polymer can be related to equivalent weight using the formula:  $50 IXR + 178 = EW$ .

The FSA polymers can be prepared as colloidal aqueous dispersions. They may also be in the form of dispersions in other media, examples of which include, but are not limited to, alcohol, water-soluble ethers, such as tetrahydrofuran, mixtures of water-soluble ethers, and combinations thereof. In making the dispersions, the polymer can be used in acid form. U.S. Pat. Nos. 4,433,082, 6,150,426 and WO 03/006537 disclose methods for making of aqueous alcoholic dispersions. After the dispersion is made, concentration and the dispersing liquid composition can be adjusted by methods known in the art.

Aqueous dispersions of the colloid-forming polymeric acids, including FSA polymers, typically have particle sizes as small as possible and an EW as small as possible, so long as a stable colloid is formed.

Aqueous dispersions of FSA polymer are available commercially as Nafion® dispersions, from E. I. du Pont de Nemours and Company (Wilmington, Del.).

#### 4. Preparation of Conductive Compositions

The new electrically conductive copolymer composition is prepared by (i) forming the electrically conductive polymer doped with a wettable FAP; (ii) forming the electrically conductive polymer doped with a non-wettable FAP; and (iii) blending the two doped conductive polymers to form the admixture.

##### (i) and (ii) Preparing Doped Electrically Conductive Polymers

In one embodiment, the doped electrically conductive polymers are formed by oxidative polymerization of the precursor monomer in the presence of the wettable FAP or non-wettable FAP, referred to generically as "FAP". The polymerization is generally carried out in a homogeneous aqueous solution. In another embodiment, the polymerization for obtaining the electrically conducting polymer is carried out in an emulsion of water and an organic solvent. In general, some water is present in order to obtain adequate solubility of the oxidizing agent and/or catalyst. Oxidizing agents such as ammonium persulfate, sodium persulfate, potassium persulfate, and the like, can be used. A catalyst, such as ferric chloride, or ferric sulfate may also be present. The resulting polymerized product will be a solution, dispersion, or emulsion of the doped conductive polymer.

In one embodiment, the method of making an aqueous dispersion of the conductive polymer doped with FAP includes forming a reaction mixture by combining water, at least one precursor monomer, at least one FAP, and an oxidizing agent, in any order, provided that at least a portion of the FAP is present when at least one of the precursor monomer and the oxidizing agent is added. It will be understood that, in the case of electrically conductive copolymers, the term "at least one precursor monomer" encompasses more than one type of monomer.

In one embodiment, the method of making an aqueous dispersion of the doped conductive polymer includes forming a reaction mixture by combining water, at least one precursor monomer, at least one FAP, and an oxidizing agent, in any order, provided that at least a portion of the FAP is present when at least one of the precursor monomer and the oxidizing agent is added.

In one embodiment, the method of making the doped conductive polymer comprises:

- (a) providing an aqueous solution or dispersion of a FAP;
- (b) adding an oxidizer to the solutions or dispersion of step (a); and
- (c) adding at least one precursor monomer to the mixture of step (b).

In another embodiment, the precursor monomer is added to the aqueous solution or dispersion of the FAP prior to adding the oxidizer. Step (b) above, which is adding oxidizing agent, is then carried out.

In another embodiment, a mixture of water and the precursor monomer is formed, in a concentration typically in the range of about 0.5% by weight to about 4.0% by weight total precursor monomer. This precursor monomer mixture is added to the aqueous solution or dispersion of the FAP, and steps (b) above which is adding oxidizing agent is carried out.

In another embodiment, the aqueous polymerization mixture may include a polymerization catalyst, such as ferric sulfate, ferric chloride, and the like. The catalyst is added before the last step. In another embodiment, a catalyst is added together with an oxidizing agent.

In one embodiment, the polymerization is carried out in the presence of co-dispersing liquids which are miscible with water. Examples of suitable co-dispersing liquids include, but are not limited to ethers, alcohols, alcohol ethers, cyclic ethers, ketones, nitrates, sulfoxides, amides, and combinations thereof. In one embodiment, the co-dispersing liquid is an alcohol. In one embodiment, the co-dispersing liquid is an organic solvent selected from n-propanol, isopropanol, t-butanol, dimethylacetamide, dimethylformamide, N-methylpyrrolidone, and mixtures thereof. In general, the amount of co-dispersing liquid should be less than about 60% by volume. In one embodiment, the amount of co-dispersing liquid is less than about 30% by volume. In one embodiment, the amount of co-dispersing liquid is between 5 and 50% by volume. The use of a co-dispersing liquid in the polymerization significantly reduces particle size and improves filterability of the dispersions. In addition, buffer materials obtained by this process show an increased viscosity and films prepared from these dispersions are of high quality.

The co-dispersing liquid can be added to the reaction mixture at any point in the process.

In one embodiment, the polymerization is carried out in the presence of a co-acid which is a Brønsted acid. The acid can be an inorganic acid, such as HCl, sulfuric acid, and the like, or an organic acid, such as acetic acid or p-toluenesulfonic acid. Alternatively, the acid can be a water soluble polymeric acid such as poly(styrenesulfonic acid), poly(2-acrylamido-2-methyl-1-propanesulfonic acid, or the like, or a second fluorinated acid polymer, as described above. Combinations of acids can be used.

The co-acid can be added to the reaction mixture at any point in the process prior to the addition of either the oxidizer or the precursor monomer, whichever is added last. In one embodiment, the co-acid is added before both the precursor monomers and the fluorinated acid polymer, and the oxidizer is added last. In one embodiment the co-acid is added prior to the addition of the precursor monomers, followed by the addition of the fluorinated acid polymer, and the oxidizer is added last.

In one embodiment, the polymerization is carried out in the presence of both a co-dispersing liquid and a co-acid.

In one embodiment, a reaction vessel is charged first with a mixture of water, alcohol co-dispersing agent, and inorganic co-acid. To this is added, in order, the precursor monomer, an aqueous solution or dispersion of FAP, and an oxidizer. The oxidizer is added slowly and dropwise to prevent the formation of localized areas of high ion concentration which can destabilize the mixture. In another embodiment, precursor monomer and aqueous oxidizer solution can be added separately and simultaneously to the aqueous solution or dispersion of FAP, a co-acid, and a catalyst. The mixture is stirred and the reaction is then allowed to proceed at a controlled temperature. When polymerization is completed, the reaction mixture is treated with a strong acid cation resin, stirred and filtered; and then treated with a base anion exchange resin, stirred and filtered. Alternative orders of addition can be used, as discussed above.

In the method of making the doped conductive polymer, the molar ratio of oxidizer to total precursor monomer is generally in the range of 0.1 to 3.0; and in one embodiment is 0.4 to 1.5. The molar ratio of FAP to total precursor monomer is generally in the range of 0.2 to 10. In one embodiment, the

ratio is in the range of 1 to 5. The overall solid content is generally in the range of about 0.5% to 12% in weight percentage; and in one embodiment of about 2% to 6%. The reaction temperature is generally in the range of about 4°C. to 50°C.; in one embodiment about 20°C. to 35°C. The molar ratio of optional co-acid to precursor monomer is about 0.05 to 4. The addition time of the oxidizer influences particle size and viscosity. Thus, the particle size can be reduced by slowing down the addition speed. In parallel, the viscosity is increased by slowing down the addition speed. The reaction time is generally in the range of about 1 to about 30 hours.

(iii) Blending the Doped Conductive Polymers

The new electrically conductive polymer composition is prepared by blending the conductive polymer doped with a wettable FAP with the conductive polymer doped with a non-wettable FAP. This can be accomplished by adding an aqueous dispersion of one doped polymer to an aqueous dispersion of the other doped polymer. In one embodiment, the composition is further treated using sonication or microfluidization to ensure mixing of the components.

In one embodiment, one or both of the doped electrically conductive polymers are isolated in solid form. The solid material can be redispersed in water or in an aqueous solution or dispersion of the other component. For example, solids of electrically conductive polymer doped with a non-wettable FAP can be dispersed in an aqueous solution or dispersion of an electrically conductive polymer doped with a wettable FAP.

(iv) pH Treatment

As synthesized, the aqueous dispersions of the doped conductive polymers generally have a very low pH. It has been found that the pH can be adjusted to higher values, without adversely affecting the properties in devices. In one embodiment, the pH of the dispersion can be adjusted to about 1.5 to about 4. In one embodiment, the pH is adjusted to between 2 and 3. It has been found that the pH can be adjusted using known techniques, for example, ion exchange or by titration with an aqueous basic solution.

In one embodiment, the as-formed aqueous dispersion of doped electrically conductive polymer is contacted with at least one ion exchange resin under conditions suitable to remove any remaining decomposed species, side reaction products, and unreacted monomers, and to adjust pH, thus producing a stable, aqueous dispersion with a desired pH. In one embodiment, the as-formed doped conductive polymer dispersion is contacted with a first ion exchange resin and a second ion exchange resin, in any order. The as-formed doped conductive polymer dispersion can be treated with both the first and second ion exchange resins simultaneously, or it can be treated sequentially with one and then the other. In one embodiment, the two doped conductive polymers are combined as-synthesized, and then treated with one or more ion exchange resins.

Ion exchange is a reversible chemical reaction wherein an ion in a fluid medium (such as an aqueous dispersion) is exchanged for a similarly charged ion attached to an immobile solid particle that is insoluble in the fluid medium. The term "ion exchange resin" is used herein to refer to all such substances. The resin is rendered insoluble due to the crosslinked nature of the polymeric support to which the ion exchanging groups are attached. Ion exchange resins are classified as cation exchangers or anion exchangers. Cation exchangers have positively charged mobile ions available for exchange, typically protons or metal ions such as sodium ions. Anion exchangers have exchangeable ions which are negatively charged, typically hydroxide ions.

In one embodiment, the first ion exchange resin is a cation, acid exchange resin which can be in protonic or metal ion, typically sodium ion, form. The second ion exchange resin is a basic, anion exchange resin. Both acidic, cation including proton exchange resins and basic, anion exchange resins are contemplated for use in the practice of the invention. In one embodiment, the acidic, cation exchange resin is an inorganic acid, cation exchange resin, such as a sulfonic acid cation exchange resin. Sulfonic acid cation exchange resins contemplated for use in the practice of the invention include, for example, sulfonated styrene-divinylbenzene copolymers, sulfonated crosslinked styrene polymers, phenol-formaldehyde-sulfonic acid resins, benzene-formaldehyde-sulfonic acid resins, and mixtures thereof. In another embodiment, the acidic, cation exchange resin is an organic acid, cation exchange resin, such as carboxylic acid, acrylic or phosphorous cation exchange resin. In addition, mixtures of different cation exchange resins can be used.

In another embodiment, the basic, anionic exchange resin is a tertiary amine anion exchange resin. Tertiary amine anion exchange resins contemplated for use in the practice of the invention include, for example, tertiary-aminated styrene-divinylbenzene copolymers, tertiary-aminated crosslinked styrene polymers, tertiary-aminated phenol-formaldehyde resins, tertiary-aminated benzene-formaldehyde resins, and mixtures thereof. In a further embodiment, the basic, anionic exchange resin is a quaternary amine anion exchange resin, or mixtures of these and other exchange resins.

The first and second ion exchange resins may contact the as-formed aqueous dispersion either simultaneously, or consecutively. For example, in one embodiment both resins are added simultaneously to an as-formed aqueous dispersion of an electrically conducting polymer, and allowed to remain in contact with the dispersion for at least about 1 hour, e.g., about 2 hours to about 20 hours. The ion exchange resins can then be removed from the dispersion by filtration. The size of the filter is chosen so that the relatively large ion exchange resin particles will be removed while the smaller dispersion particles will pass through. Without wishing to be bound by theory, it is believed that the ion exchange resins quench polymerization and effectively remove ionic and non-ionic impurities and most of unreacted monomer from the as-formed aqueous dispersion. Moreover, the basic, anion exchange and/or acidic, cation exchange resins renders the acidic sites more basic, resulting in increased pH of the dispersion. In general, about one to five grams of ion exchange resin is used per gram of new conductive polymer composition.

In many cases, the basic ion exchange resin can be used to adjust the pH to the desired level. In some cases, the pH can be further adjusted with an aqueous basic solution such as a solution of sodium hydroxide, ammonium hydroxide, tetramethylammonium hydroxide, or the like.

In another embodiment, more conductive dispersions are formed by the addition of highly conductive additives to the aqueous dispersions of the new conductive polymer composition. Because dispersions with relatively high pH can be formed, the conductive additives, especially metal additives, are not attacked by the acid in the dispersion. Examples of suitable conductive additives include, but are not limited to metal particles and nanoparticles, nanowires, carbon nanotubes, graphite fibers or particles, carbon particles, and combinations thereof.

5. Buffer Layers

In another embodiment of the invention, there are provided buffer layers deposited from aqueous dispersions comprising

the new conductive polymer composition. The term "layer" is used interchangeably with the term "film" and refers to a coating covering a desired area. The term is not limited by size. The area can be as large as an entire device or as small as a specific functional area such as the actual visual display, or as small as a single sub-pixel. Layers and films can be formed by any conventional deposition technique, including vapor deposition, liquid deposition (continuous and discontinuous techniques), and thermal transfer. Continuous deposition techniques, include but are not limited to, spin coating, gravure coating, curtain coating, dip coating, slot-die coating, spray coating, and continuous nozzle coating. Discontinuous deposition techniques include, but are not limited to, ink jet printing, gravure printing, and screen printing.

In some embodiments, the dried films of the new conductive polymer composition are not redispersible in water. Thus the buffer layer can be applied as multiple thin layers. In addition, the buffer layer can be overcoated with a layer of different water-soluble or water-dispersible material without being damaged. Buffer layers comprising the new conductive polymer composition have been surprisingly found to have improved wettability.

In another embodiment, there are provided buffer layers deposited from aqueous dispersions comprising the new conductive polymer composition blended with other water soluble or dispersible materials. Examples of types of materials which can be added include, but are not limited to polymers, dyes, coating aids, organic and inorganic conductive inks and pastes, charge transport materials, crosslinking agents, and combinations thereof. The other water soluble or dispersible materials can be simple molecules or polymers. Examples of suitable polymers include, but are not limited to, conductive polymers such as polythiophenes, polyanilines, polypyrroles, polyacetylenes, and combinations thereof.

#### 6. Electronic Devices

In another embodiment of the invention, there are provided electronic devices comprising at least one electroactive layer positioned between two electrical contact layers, wherein the device further includes the new buffer layer. The term "electroactive" when referring to a layer or material is intended to mean a layer or material that exhibits electronic or electro-radiative properties. An electroactive layer material may emit radiation or exhibit a change in concentration of electron-hole pairs when receiving radiation.

As shown in FIG. 2, a typical device, 100, has an anode layer 110, a buffer layer 120, an electroactive layer 130, and a cathode layer 150. Adjacent to the cathode layer 150 is an optional electron-injection/transport layer 140.

The device may include a support or substrate (not shown) that can be adjacent to the anode layer 110 or the cathode layer 150. Most frequently, the support is adjacent the anode layer 110. The support can be flexible or rigid, organic or inorganic. Examples of support materials include, but are not limited to, glass, ceramic, metal, and plastic films.

The anode layer 110 is an electrode that is more efficient for injecting holes compared to the cathode layer 150. The anode can include materials containing a metal, mixed metal, alloy, metal oxide or mixed oxide. Suitable materials include the mixed oxides of the Group 2 elements (i.e., Be, Mg, Ca, Sr, Ba, Ra), the Group 11 elements, the elements in Groups 4, 5, and 6, and the Group 8-10 transition elements. If the anode layer 110 is to be light transmitting, mixed oxides of Groups 12, 13 and 14 elements, such as indium-tin-oxide, may be used. As used herein, the phrase "mixed oxide" refers to oxides having two or more different cations selected from the Group 2 elements or the Groups 12, 13, or 14 elements. Some

non-limiting, specific examples of materials for anode layer 110 include, but are not limited to, indium-tin-oxide ("ITO"), indium-zinc-oxide, aluminum-tin-oxide, gold, silver, copper, and nickel. The anode may also comprise an organic material, especially a conducting polymer such as polyaniline, including exemplary materials as described in "Flexible light-emitting diodes made from soluble conducting polymer," Nature vol. 357, pp 477-479 (11 Jun. 1992). At least one of the anode and cathode should be at least partially transparent to allow the generated light to be observed.

The anode layer 110 may be formed by a chemical or physical vapor deposition process or spin-cast process. Chemical vapor deposition may be performed as a plasma-enhanced chemical vapor deposition ("PECVD") or metal organic chemical vapor deposition ("MOCVD"). Physical vapor deposition can include all forms of sputtering, including ion beam sputtering, as well as e-beam evaporation and resistance evaporation. Specific forms of physical vapor deposition include rf magnetron sputtering and inductively-coupled plasma physical vapor deposition ("IMP-PVD"). These deposition techniques are well known within the semiconductor fabrication arts.

In one embodiment, the anode layer 110 is patterned during a lithographic operation. The pattern may vary as desired. The layers can be formed in a pattern by, for example, positioning a patterned mask or resist on the first flexible composite barrier structure prior to applying the first electrical contact layer material. Alternatively, the layers can be applied as an overall layer (also called blanket deposit) and subsequently patterned using, for example, a patterned resist layer and wet chemical or dry etching techniques. Other processes for patterning that are well known in the art can also be used.

The buffer layer 120 is usually deposited onto substrates using a variety of techniques well-known to those skilled in the art. Typical deposition techniques, as discussed above, include vapor deposition, liquid deposition (continuous and discontinuous techniques), and thermal transfer.

An optional layer, not shown, may be present between the buffer layer 120 and the electroactive layer 130. This layer 40 may comprise hole transport materials. Examples of hole transport materials for layer 120 have been summarized for example, in Kirk-Othmer Encyclopedia of Chemical Technology, Fourth Edition, Vol. 18, p. 837-860, 1996, by Y. Wang. Both hole transporting molecules and polymers can be used. 45 Commonly used hole transporting molecules include, but are not limited to: 4,4',4"-tris(N,N-diphenyl-amino)-triphenylamine (TDATA); 4,4',4"-tris(N-3-methylphenyl-N-phenyl-amino)-triphenylamine (MTDATA); N,N'-diphenyl-N,N'-bis(3-methylphenyl)-[1,1'-biphenyl]4,4'-diamine (TPD); 1,1-bis[(di-4-tolylamino) phenyl]cyclohexane (TAPC); N,N'-bis(4-methylphenyl)-N,N'-bis(4-ethylphenyl)-[1,1'-(3,3'-dimethyl)biphenyl]4,4'-diamine (ETPD); tetrakis(3-methylphenyl)-N,N,N',N'-2,5-phenylenediamine (PDA);  $\alpha$ -phenyl-4-N,N-diphenylaminostyrene (TPS); p-(diethylamino)benzaldehyde diphenylhydrazone (DEH); triphenylamine (TPA); bis[4-(N,N-diethylamino)-2-methylphenyl](4-methylphenyl)methane (MPMP); 1-phenyl-3-[p-(diethylamino)styryl]-5-[p-(diethylamino)phenyl]pyrazoline (PPR or DEASP); 1,2-trans-bis(9H-carbazol-9-yl)cyclobutane (DCZB); N,N,N',N'-tetrakis(4-methylphenyl)-(1,1'-biphenyl)4,4'-diamine (TTB); N,N'-bis(naphthalen-1-yl)-N,N'-bis-(phenyl)benzidine ( $\alpha$ -NPB); and porphyrinic compounds, such as copper phthalocyanine. Commonly used hole transporting polymers include, but are not limited to, poly(9,9-diptylfluorene-co-N-(4-butylphenyl)diphenylamine), and the like, polyvinylcarbazole, (phenylmethyl)polysilane, poly(dioxythiophenes), polyanilines, 55 60 65 70 75 80 85 90 95

and polypyroroles. It is also possible to obtain hole transporting polymers by doping hole transporting molecules such as those mentioned above into polymers such as polystyrene and polycarbonate.

Depending upon the application of the device, the electroactive layer 130 can be a light-emitting layer that is activated by an applied voltage (such as in a light-emitting diode or light-emitting electrochemical cell), a layer of material that responds to radiant energy and generates a signal with or without an applied bias voltage (such as in a photodetector). In one embodiment, the electroactive material is an organic electroluminescent ("EL") material. Any EL material can be used in the devices, including, but not limited to, small molecule organic fluorescent compounds, fluorescent and phosphorescent metal complexes, conjugated polymers, and mixtures thereof. Examples of fluorescent compounds include, but are not limited to, pyrene, perylene, rubrene, coumarin, derivatives thereof, and mixtures thereof. Examples of metal complexes include, but are not limited to, metal chelated oxinoid compounds, such as tris(8-hydroxyquinolato)aluminum (Alq<sub>3</sub>); cyclometalated iridium and platinum electroluminescent compounds, such as complexes of iridium with phenylpyridine, phenylquinoline, or phenylpyrimidine ligands as disclosed in Petrov et al., U.S. Pat. No. 6,670,645 and Published PCT Applications WO 03/063555 and WO 2004/016710, and organometallic complexes described in, for example, Published PCT Applications WO 03/008424, WO 03/091688, and WO 03/040257, and mixtures thereof. Electroluminescent emissive layers comprising a charge carrying host material and a metal complex have been described by Thompson et al., in U.S. Pat. No. 6,303,238, and by Burrows and Thompson in published PCT applications WO 00/70655 and WO 01/41512. Examples of conjugated polymers include, but are not limited to poly(phenylenevinylene), polyfluorenes, poly(spirofluorenes), polythiophenes, poly(p-phenylenes), copolymers thereof, and mixtures thereof.

Optional layer 140 can function both to facilitate electron injection/transport, and can also serve as a confinement layer to prevent quenching reactions at layer interfaces. More specifically, layer 140 may promote electron mobility and reduce the likelihood of a quenching reaction if layers 130 and 150 would otherwise be in direct contact. Examples of materials for optional layer 140 include, but are not limited to, metal chelated oxinoid compounds, such as bis(2-methyl-8-quinolinolato)(para-phenyl-phenolato)aluminum(III) (BAIQ), tetra(8-hydroxyquinolato)zirconium (ZrQ), and tris(8-hydroxyquinolato)aluminum (Alq<sub>3</sub>); azole compounds such as 2-(4-biphenyl)-5-(4-t-butylphenyl)-1,3,4-oxadiazole (PBD), 3-(4-biphenyl)4-phenyl-5-(4-t-butylphenyl)-1,2,4-triazole (TAZ), and 1,3,5-tri(phenyl-2-benzimidazolyl)benzene (TPBI); quinoxaline derivatives such as 2,3-bis(4-fluorophenyl)quinoxaline; phenanthroline derivatives such as 9,10-diphenylphenanthroline (DPA) and 2,9-dimethyl-4,7-diphenyl-1,10-phenanthroline (DDPA); and any one or more combinations thereof. Alternatively, optional layer 140 may be inorganic and comprise BaO, LiF, Li<sub>2</sub>O, or the like.

The cathode layer 150 is an electrode that is particularly efficient for injecting electrons or negative charge carriers. The cathode layer 150 can be any metal or nonmetal having a lower work function than the first electrical contact layer (in this case, the anode layer 110). As used herein, the term "lower work function" is intended to mean a material having a work function no greater than about 4.4 eV. As used herein, "higher work function" is intended to mean a material having a work function of at least approximately 4.4 eV.

Materials for the cathode layer can be selected from alkali metals of Group 1 (e.g., Li, Na, K, Rb, Cs,), the Group 2 metals (e.g., Mg, Ca, Ba, or the like), the Group 12 metals, the lanthanides (e.g., Ce, Sm, Eu, or the like), and the actinides (e.g., Th, U, or the like). Materials such as aluminum, indium, yttrium, and combinations thereof, may also be used. Specific non-limiting examples of materials for the cathode layer 150 include, but are not limited to, barium, lithium, cerium, cesium, europium, rubidium, yttrium, magnesium, samarium, and alloys and combinations thereof.

The cathode layer 150 is usually formed by a chemical or physical vapor deposition process. In some embodiments, the cathode layer will be patterned, as discussed above in reference to the anode layer 110.

Other layers in the device can be made of any materials which are known to be useful in such layers upon consideration of the function to be served by such layers.

In some embodiments, an encapsulation layer (not shown) is deposited over the contact layer 150 to prevent entry of undesirable components, such as water and oxygen, into the device 100. Such components can have a deleterious effect on the organic layer 130. In one embodiment, the encapsulation layer is a barrier layer or film. In one embodiment, the encapsulation layer is a glass lid.

Though not depicted, it is understood that the device 100 may comprise additional layers. Other layers that are known in the art or otherwise may be used. In addition, any of the above-described layers may comprise two or more sub-layers or may form a laminar structure. Alternatively, some or all of anode layer 110, the buffer layer 120, the electron transport layer 140, cathode layer 150, and other layers may be treated, especially surface treated, to increase charge carrier transport efficiency or other physical properties of the devices. The choice of materials for each of the component layers is preferably determined by balancing the goals of providing a device with high device efficiency with device operational lifetime considerations, fabrication time and complexity factors and other considerations appreciated by persons skilled in the art. It will be appreciated that determining optimal components, component configurations, and compositional identities would be routine to those of ordinary skill of in the art.

In various embodiments, the different layers have the following ranges of thicknesses: anode 110, 500-5000 Å, in one embodiment 1000-2000 Å; buffer layer 120, 50-2000 Å, in one embodiment 200-1000 Å; optional transport layer, 50-2000 Å, in one embodiment 100-1000 Å; photoactive layer 130, 10-2000 Å, in one embodiment 100-1000 Å; optional electron transport layer 140, 50-2000 Å, in one embodiment 100-1000 Å; cathode 150, 200-10000 Å, in one embodiment 300-5000 Å. The location of the electron-hole recombination zone in the device, and thus the emission spectrum of the device, can be affected by the relative thickness of each layer. Thus the thickness of the electron-transport layer should be chosen so that the electron-hole recombination zone is in the light-emitting layer. The desired ratio of layer thicknesses will depend on the exact nature of the materials used.

In operation, a voltage from an appropriate power supply (not depicted) is applied to the device 100. Current therefore passes across the layers of the device 100. Electrons enter the organic polymer layer, releasing photons. In some OLEDs, called active matrix OLED displays, individual deposits of photoactive organic films may be independently excited by the passage of current, leading to individual pixels of light emission. In some OLEDs, called passive matrix OLED dis-

plays, deposits of photoactive organic films may be excited by rows and columns of electrical contact layers.

As used herein, the terms "comprises," "comprising," "includes," "including," "has," "having" or any other variation thereof, are intended to cover a non-exclusive inclusion. For example, a process, method, article, or apparatus that comprises a list of elements is not necessarily limited to only those elements but may include other elements not expressly listed or inherent to such process, method, article, or apparatus. Further, unless expressly stated to the contrary, "or" refers to an inclusive or and not to an exclusive or. For example, a condition A or B is satisfied by any one of the following: A is true (or present) and B is false (or not present), A is false (or not present) and B is true (or present), and both A and B are true (or present).

Also, use of "a" or "an" are employed to describe elements and components of the invention. This is done merely for convenience and to give a general sense of the invention. This description should be read to include one or at least one and the singular also includes the plural unless it is obvious that it is meant otherwise.

The term "hole transport" when referring to a layer, material, member, or structure, is intended to mean such layer, material, member, or structure facilitates migration of positive charges through the thickness of such layer, material, member, or structure with relative efficiency and small loss of charge.

The term "electron transport" means when referring to a layer, material, member or structure, such a layer, material, member or structure that promotes or facilitates migration of negative charges through such a layer, material, member or structure into another layer, material, member or structure.

The term "organic electronic device" is intended to mean a device including one or more semiconductor layers or materials. Organic electronic devices include, but are not limited to: (1) devices that convert electrical energy into radiation (e.g., a light-emitting diode, light emitting diode display, diode laser, or lighting panel), (2) devices that detect signals through electronic processes (e.g., photodetectors photoconductive cells, photoresistors, photoswitches, phototransistors, phototubes, infrared ("IR") detectors, or biosensors), (3) devices that convert radiation into electrical energy (e.g., a photovoltaic device or solar cell), and (4) devices that include one or more electronic components that include one or more organic semiconductor layers (e.g., a transistor or diode).

Unless otherwise defined, all technical and scientific terms used herein have the same meaning as commonly understood by one of ordinary skill in the art to which this invention belongs. In the Formulae, the letters Q, R, T, W, X, Y, and Z are used to designate atoms or groups which are defined within. All other letters are used to designate conventional atomic symbols. Group numbers corresponding to columns within the Periodic Table of the elements use the "New Notation" convention as seen in the *CRC Handbook of Chemistry and Physics*, 81<sup>st</sup> Edition (2000).

Although methods and materials similar or equivalent to those described herein can be used in the practice or testing of the present invention, suitable methods and materials are described below. All publications, patent applications, patents, and other references mentioned herein are incorporated by reference in their entirety. In case of conflict, the present specification, including definitions, will control. In addition, the materials, methods, and examples are illustrative only and not intended to be limiting.

It is to be appreciated that certain features of the invention which are, for clarity, described above and below in the context of separate embodiments, may also be provided in com-

bination in a single embodiment. Conversely, various features of the invention that are, for brevity, described in the context of a single embodiment, may also be provided separately or in any subcombination. Further, reference to values stated in ranges includes each and every value within that range.

## EXAMPLES

### Example 1

This example illustrates the preparation of an aqueous dispersion of an electrically conductive polymer doped with a non-wettable FAP. The conductive polymer is polyaniline. The non-wettable FAP is Nafion®, a polyperfluoroethylene/perfluoroethersulfoic acid, which is a colloid forming acid. The doped conductive polymer is polyaniline/Nafion®.

A small drop of the Nafion® was cast on a microscope slide. The film was dried at ~90° C. in a vacuum oven. A small drop of p-xylene was placed on the dried film of the Nafion®. The liquid formed a ball-like droplet and rolled around easily. A film of Nafion® will not be wettable by phenylhexane, and the contact angle will be greater than 40°.

455.83 g of DI water and 440.86 g of 99.7% n-propanol were massed directly into a 2 L glass reactor vessel at room temperature. Next, 0.942 mL (11.49 mmol) of 37% wt. HCl and 6.29 mL (68.96 mmol) of aniline (distilled) were added to the reactor via pipet. The mixture was stirred overhead with a U-shaped stir-rod set at 350 RPM. After seven minutes, 479.37 (57.46 mmol) of water-dispersed Nafion® (DE-1020, 11.4% solids, 951.0 EW) that had been passed through a 0.3 µm profile filter, was added slowly via glass funnel. The mixture was allowed to homogenize for an additional 17 minutes. 16.39 (71.83 mmol) of ammonium persulfate (99.99+%) dissolved in 100 g of DI water was added drop-wise at 8.34 ml/hr to the reactants via syringe infusion pump. Five minutes later the solution turned light turquoise. The solution progressed to being dark blue before turning very dark green. After completion of APS addition, the mixture was stirred for additional one hour before addition of 35 of Amberlyst-15 (Rohm and Haas Co., Philadelphia, Pa.) cation exchange resin (rinsed multiple times with a 32% n-propanol/DI water mixture and dried under nitrogen) was added and the stirring commenced overnight at 150 RPM. The next morning, the mixture was filtered through steel mesh and stirred with Amberjet 4400(OH) (Rohm and Haas Co., Philadelphia, Pa.) anion exchange resin (rinsed multiple times with a 32% n-propanol (in DI water) mixture and dried under nitrogen) until the pH had changed from 1.35 to 5.8. The resin was again filtered off and the filtrate is a stable dispersion. Solid % of the dispersion is about 4%(w/w).

### Example 2

This example illustrates the properties and device performance of Polyaniline/Nafion®:

The dispersion made in Example 1 was filtered through a 0.45 µm Millipore Millex-HV syringe filter with PVDF membrane. The dispersions were spun onto glass at 1,000 RPM, resulting in films having a thickness of ~2,200 Å. The conductivity was measured to be  $4.0 \times 10^{-5}$  S/cm at ambient temperature.

The dispersion was also spin-coated to form a thin film for measurement of contact angle. The measurement is described below. A goniometer was used to dispense 3.0 µL drops of phenylhexane. Once a drop was dispensed, a snapshot was immediately taken, giving a visual outline of the drop. Each measurement calculated a right and left value for the contact

angle. It was determined to be 57 degrees. This contact angle is very high, indicating that its film surface is difficult to wet with organic solvents such as p-xylene, toluene. The solvents are common ones for dissolving light emitting materials.

The polyaniline/Nafion® was then tested for device performance. The dispersion was spun on a 6"×6" glass plate. The plate had an ITO thickness of 100 to 150 nm and consisted of 16 backlight substrates. Each substrate consisted of 3 pieces of 5 mm×5 mm pixel and 1 piece of 2 mm×2 mm pixel for light emission. The spin-coated films as buffer layer layers were then baked at 130° C. for 5 minutes on a hot plate in air. The thickness of the baked buffer layers was about 80 nm. For the light-emitting layer, a 1% (w/v) toluene solution of a green polyfluorene light-emitting polymer was spin-coated on top of the buffer layer films and subsequently baked at 130° C. for 10 minutes on a hot plate in an inert atmosphere dry box. The thickness of the baked films was 75 nm. Immediately after, a 3 nm thick barium layer and a 350-400 nm aluminum layer were deposited on the green light-emitting polymer films to serve as a cathode. The device data of this example is shown in Table 1 along with pH of the dispersion, conductivity and contact angle. The data shows that polyaniline/Nafion® has a higher contact angle and lower conductivity compared to polyaniline/poly(VF2/PSEBVE acid). The high contact angle renders the surface more difficult to wet with common organic solvents for light emitting materials. Although the devices made with polyaniline/Nafion® as a buffer layer have lower voltage, higher efficiency, but have lower device lifetime compared to the devices made with polyaniline/poly(VF2/PSEBVE acid), which will be illustrated in Example 5.

### Example 3

This example illustrates the preparation of an organic solvent wettable fluorinated acid polymer, VF<sub>2</sub>/PSEBVE Copolymer, converted to the sulfonic acid form.

## GLOSSARY



2-(1,1-difluoro-2-(trifluoromethyl)allyloxy)-  
1,1,2,2-tetrafluoroethanesulfonyl fluoride  
(PSEBVE)

-continued



5

15

20 (0.42 mol). The vessel was cooled to  $-35^{\circ}\text{C}.$ , evacuated to  $-3$  PSIG, and purged with nitrogen. The evacuate/purge cycle was repeated two more times. To the vessel was then added 29 VF<sub>2</sub> (0.45 mol). The vessel was heated to  $28^{\circ}\text{C}.$ , which increased the pressure to 92 PSIG. The reaction temperature 25 was maintained at  $28^{\circ}\text{C}.$  for 18 h. at which time the pressure had dropped to 32 PSIG. The vessel was vented and the crude liquid material was recovered. The Vertrel® XF was removed in vacuo to afford 110 g of desired copolymer. Conversion of 30 the sulfonyl fluoride copolymer prepared above to sulfonic acid was carried out in the following manner. 20 of dried polymer and 5.0 g lithium carbonate were refluxed in 100 mL dry methanol for 12 h. The mixture was brought to room temperature and filtered to remove any remaining solids. The methanol was removed in vacuo to isolate the lithium salt of 35 the polymer. The lithium salt of the polymer was then dissolved in water and added with Amberlyst 15, a protonic acid exchange resin which had been washed thoroughly with water until there was no color in the water. The mixture was stirred and filtered. Filtrate was added with fresh Amberlyst 40 15 resin and filtered again. The step was repeated two more times. Water was then removed from the final filtrates and the solids were then dried in a vacuum oven.

#### Example 4

45

This example illustrates the preparation of Polyaniline/Poly(VF2-PSEBVE acid).

78.61 g of deionized water and 45.38 g of 99.7% n-propanol were massed directly into a 1,000 mL reactor vessel at room temperature. Next, 0.0952 mL (1.2 mmol) of 37% wt. HCl and 0.6333 mL (7.0 mmol) of aniline (distilled) were added to the reactor via pipet. The mixture was stirred overhead with a U-shaped stir-rod set at 100 RPM. After five minutes, 53.60 g of 4.39% water solution of the polymer (5.80 mmol) made in Example 1 (10.90 mmol) was added slowly via a glass funnel. The mixture was allowed to homogenize at 200 rpm for an additional 10 minutes. 1.65 g (7.2 mmol) of ammonium persulfate (99.99+% dissolved in 20 of DI water was added drop wise to the reactants via syringe infusion pump in six hours. Eight minutes later the solution turned light turquoise. The solution progressed to being dark blue before turning very dark green. After the APS addition, the mixture was stirred for 60 minutes and 4.68 g of Amberlyst-15 (Rohm and Haas Co., Philadelphia, Pa.) cation exchange resin (rinsed multiple times with a 32% n-propanol/DI water mixture and dried under nitrogen) was added and the stirring commenced overnight at 200 RPM. The next morning, the

31

mixture was filtered through steel mesh. pH of the Amberlyst 15 treated dispersion was 1.2. Portion of the dispersion was stirred with Amberjet 4400 (OH) (Rohm and Haas Co., Philadelphia, Pa.) anion exchange resin (rinsed multiple times with a 32% n-propanol/DI water mixture and dried under nitrogen) until the pH had changed from 1.2 to 5.7. The resin was again filtered off and the filtrate is a stable dispersion. Solid % of the dispersion is about 1.5% (w/w).

## Example 5

The examples illustrates the properties and device performance of Polyaniline/Poly(VF2/PSEBVE acid)

The dispersion made in Example 4 was filtered through a 0.45  $\mu\text{m}$  Millipore Millex-HV syringe filter with PVDF membrane. The dispersions were spun onto glass at 1,000 RPM for 80 seconds, resulting in films having a thickness of 831  $\text{\AA}$  once baked at 130° C. for 5 minutes in air and further baked at 200° C. for 10 minutes in glove box for minutes. Conductivity was measured to be  $4.0 \times 10^{-4}$  S/cm. The dispersion was also spin-coated to thin film for measurement of contact angle. The measurement is described in Example 2 and the film surface was measured to have contact angle of 20 degree. This contact angle is very low, indicating that its film surface is easy to wet with the organic solvents such as p-xylene, toluene. The solvents are common for dissolving light emitting materials.

The polyaniline/poly(VF2/PSEBVE acid) was then tested for device performance. The dispersion was spun on a 6" x 6" glass plate. The plate had an ITO thickness of 100 to 150 nm and consisted of 16 backlight substrates. Each substrate consisted of 3 pieces of 5 mm x 5 mm pixel and 1 piece of 2 mm x 2 mm pixel for light emission. The spin-coated films as buffer layer layers were then baked at 130° C. for 5 minutes on a hot plate in air. The thickness of the baked buffer layers was about 80 nm. For light-emitting layer, a 1% (w/v) toluene solution of a green polyfluorene-based light-emitting polymer was spin-coated on top of the buffer layer films and subsequently baked at 130° C. for 10 minutes on a hot plate in an inert atmosphere dry box. The thickness of the baked films was 75 nm. Immediately after, a 3 nm thick barium layer and a 350-400 nm aluminum layer were deposited on the green light-emitting polymer films to serve as a cathode. The device data of this example is shown In Table 1 along with pH of the dispersion, conductivity and contact angle. The data shows that polyaniline/poly(VF2/PSEBVE acid) film surface has a much lower contact angle and higher conductivity compared to polyaniline/Nafion®. The low contact and high conductivity are desired, but the devices made with polyaniline/poly (VF2/PSEBVE acid) as a buffer layer have slightly higher voltage and lower efficiency although it has higher device lifetime compared to the devices made with polyaniline/Nafion®, which is described in Example 3.

## Example 6

This example illustrates the properties and device performance of a conductive polymer composition which is an admixture of a conductive polymer doped with a wettable FSA and a conductive polymer doped with a non-wettable FSA. The conductive polymer composition is a blend of Polyaniline/Poly(VF2/PSEBVE acid) and Polyaniline/Nafion®. This example illustrates reduced contact angle and combined performance of positive device properties by blending polyaniline/poly(VF2/PSEBVE acid) and polyaniline/Nafion®.

32

10.8 polyaniline/Nafion® made in Example 1 was mixed with 29.1 g polyaniline/poly(VF2/PSEBVE acid) made in Example 4. The mixture was stirred on a roller for several hours before use. The mixture was a stable dispersion and formed a smooth, homogeneous film upon drying. The first qualitative test showed that the film could be wetted much easily with p-xylene or toluene than the film cast from polyaniline/Nafion®.

10 The dispersions were spun onto glass and then baked at 130° C. for 45 minutes in air. Conductivity was measured to be  $7.9 \times 10^{-4}$  S/cm. The dispersion was also spin-coated to thin film for measurement of contact angle. The measurement is described in Example 2 and the film surface was measured to have contact angle of 44 degree. This contact angle is much lower than that of polyaniline/Nafion® film. This result agrees with the qualitative test described above, indicating that the dried film surface of the blend is easy to wet with the organic solvents such as p-xylene, toluene. The solvents are 15 common for dissolving light emitting materials.

15 The dispersion blend of polyaniline/poly(VF2/PSEBVE acid) and polyaniline/Nafion® was then tested for device performance. The dispersion was spun on a 6" x 6" glass plate. The plate had an ITO thickness of 100 to 150 nm and consisted of 16 backlight substrates. Each substrate consisted of 25 3 pieces of 5 mm x 5 mm pixel and 1 piece of 2 mm x 2 mm pixel for light emission. The spin-coated films as buffer layer layers were then baked at 130° C. for 5 minutes on a hot plate in air. The thickness of the baked buffer layers was about 80 nm. For light-emitting layer, a 1% (w/v) toluene solution of a green polyfluorene-based light-emitting polymer was spin-coated on top of the buffer layer films and subsequently baked at 130° C. for 10 minutes on a hot plate in an inert atmosphere dry box. The thickness of the baked films was 75 nm. Immediately after, a 3 nm thick barium layer and a 350-400 nm aluminum layer were deposited on the green light-emitting polymer films to serve as a cathode. The device data of this example is shown In Table 1 along with pH of the dispersion, 30 conductivity and contact angle. The data shows that the polymer blend has a much lower contact angle and higher conductivity than polyaniline/Nafion®. The low contact angle and high conductivity are desired. The devices made with the polymer blend as a buffer layer has higher efficiency than and 35 lower voltage than those of polyaniline/poly(VF2/PSEBVE acid). Moreover, it has a much higher device operation lifetime than polyaniline/Nafion®.

TABLE 1

| Comparative data of conductivity, contact angle and device performance |                      |                      |                      |
|------------------------------------------------------------------------|----------------------|----------------------|----------------------|
|                                                                        | Buffer               |                      |                      |
|                                                                        | Example 2            | Example 5            | Example 6            |
| pH                                                                     | 5.9                  | 5.7                  | 5.7                  |
| Lifetime (hrs) @ 5,000nits                                             | 380                  | 500 to 600           | 600 to 650           |
| Efficiency (cd/A) @ 1,000nits                                          | 16                   | 10.5                 | 14.2                 |
| Voltage (V) @ 1,000nits                                                | 2.8                  | 3.3                  | 3                    |
| Conductivity (S/cm)                                                    | $4.0 \times 10^{-5}$ | $4.0 \times 10^{-4}$ | $7.9 \times 10^{-5}$ |
| Contact Angle (degree)                                                 | 57                   | 20                   | 44                   |

55 Note that not all of the activities described above in the general description or the examples are required, that a portion of a specific activity may not be required, and that one or more further activities may be performed in addition to those described. Still further, the order in which activities are listed 60 are not necessarily the order in which they are performed.

## 33

In the foregoing specification, the concepts have been described with reference to specific embodiments. However, one of ordinary skill in the art appreciates that various modifications and changes can be made without departing from the scope of the invention as set forth in the claims below. Accordingly, the specification and figures are to be regarded in an illustrative rather than a restrictive sense, and all such modifications are intended to be included within the scope of invention. 5

Benefits, other advantages, and solutions to problems have been described above with regard to specific embodiments. However, the benefits, advantages, solutions to problems, and any feature(s) that may cause any benefit, advantage, or solution to occur or become more pronounced are not to be construed as a critical, required, or essential feature of any or all 10 claims.

It is to be appreciated that certain features are, for clarity, described herein in the context of separate embodiments, may also be provided in combination in a single embodiment. Conversely, various features that are, for brevity, described in the context of a single embodiment, may also be provided separately or in any subcombination. Further, reference to values stated in ranges includes each and every value within that range subcombination. Further, reference to values stated in ranges include each and every value within that range. 15

What is claimed is:

1. An electrically conductive polymer composition comprising a first electrically conductive polymer doped with an organic solvent wettable fluorinated acid polymer in admixture with a second electrically conductive polymer doped with an organic solvent non-wettable fluorinated acid polymer. 30

2. An electrically conductive polymer composition of claim 1 wherein each first electrically conductive polymer comprises one or more independently substituted or unsubstituted monomers selected from thiophenes, pyrroles, anilines, fused polycyclic heteroaromatics, and polycyclic heteroaromatics. 35

3. An electrically conductive polymer composition of claim 2 wherein the thiophenes have structure represented by formulas selected from Formula I and Formula Ia: 40



(I)

50

wherein:

R¹ is independently selected so as to be the same or different at each occurrence and is selected from hydrogen, alkyl, alkenyl, alkoxy, alkanoyl, alkythio, aryloxy, alkylthioalkyl, alkylaryl, arylalkyl, amino, alkylamino, dialkylamino, aryl, alkylsulfinyl, alkoxyalkyl, alkylsulfonyl, arylthio, arylsulfinyl, alkoxy carbonyl, arylsulfonyl, acrylic acid, phosphoric acid, phosphonic acid, halogen, nitro, cyano, hydroxyl, epoxy, silane, siloxane, alcohol, benzyl, carboxylate, ether, amidosulfonate, ether carboxylate, ether sulfonate, ester sulfonate, and urethane; or both R¹ groups together may form an alkylene or alkenylene chain completing a 3, 4, 5, 6, or 7-membered aromatic or alicyclic ring, which ring may optionally include one or more divalent nitrogen, sulfur or oxygen atoms; and 55

## 34

or alicyclic ring, which ring may optionally include one or more divalent nitrogen, sulfur or oxygen atoms; and



(Ia)

wherein:

R⁷ is the same or different at each occurrence and is selected from hydrogen, alkyl, heteroalkyl, alkenyl, heteroalkenyl, alcohol, amidosulfonate, benzyl, carboxylate, ether, ether carboxylate, ether sulfonate, ester sulfonate, and urethane, with the proviso that at least one R⁷ is not hydrogen, and

m is 2 or 3.

4. An electrically conductive polymer composition of claim 2 wherein the pyrroles have structure represented by Formula II:



(II)

wherein:

R¹ is independently selected so as to be the same or different at each occurrence and is selected from hydrogen, alkyl, alkenyl, alkoxy, alkanoyl, alkythio, aryloxy, alkylthioalkyl, alkylaryl, arylalkyl, amino, alkylamino, dialkylamino, aryl, alkylsulfinyl, alkoxyalkyl, alkylsulfonyl, arylthio, arylsulfinyl, alkoxy carbonyl, arylsulfonyl, acrylic acid, phosphoric acid, phosphonic acid, halogen, nitro, cyano, hydroxyl, epoxy, silane, siloxane, alcohol, benzyl, carboxylate, ether, amidosulfonate, ether carboxylate, ether sulfonate, ester sulfonate, and urethane; or both R¹ groups together may form an alkylene or alkenylene chain completing a 3, 4, 5, 6, or 7-membered aromatic or alicyclic ring, which ring may optionally include one or more divalent nitrogen, sulfur or oxygen atoms; and

R² is independently selected so as to be the same or different at each occurrence and is selected from hydrogen, alkyl, alkenyl, aryl, alkanoyl, alkylthioalkyl, alkylaryl, arylalkyl, amino, epoxy, silane, siloxane, alcohol, benzyl, carboxylate, ether, ether carboxylate, ether sulfonate, ester sulfonate, and urethane.

5. An electrically conductive polymer composition of claim 2 wherein the anilines have structure represented by formulas selected from Formula III, Formula IVa, and Formula IVb:



(III)

5

wherein:

a is 0 or an integer from 1 to 4;

b is an integer from 1 to 5, with the proviso that a+b=5; and

R<sup>1</sup> is independently selected so as to be the same or different at each occurrence and is selected from hydrogen, alkyl, alkenyl, alkoxy, alkanoyl, alkylthio, aryloxy, alkylthioalkyl, alkylaryl, arylalkyl, amino, alkylamino, dialkylamino, aryl, alkylsulfinyl, alkoxyalkyl, alkylsulfonyl, arylthio, arylsulfinyl, alkoxy carbonyl, arylsulfonyl, acrylic acid, phosphoric acid, phosphonic acid, halogen, nitro, nitrile, cyano, hydroxyl, epoxy, silane, siloxane, alcohol, benzyl, carboxylate, ether, ether carboxylate, amidosulfonate, ether sulfonate, ester sulfonate, and urethane; or both R<sup>1</sup> groups together may form an alkenylene or alkenylene chain completing a 5 or 6-membered 15 aromatic ring, which ring may optionally include one or more divalent nitrogen, sulfur or oxygen atoms; and

## 36

alkoxyalkyl, alkylsulfonyl, arylthio, arylsulfinyl, alkoxy carbonyl, arylsulfonyl, acrylic acid, phosphoric acid, phosphonic acid, halogen, nitro, nitrile, cyano, hydroxyl, epoxy, silane, siloxane, alcohol, benzyl, carboxylate, ether, ether carboxylate, amidosulfonate, ether sulfonate, ester sulfonate, and urethane; and

at least one of R<sup>8</sup> and R<sup>9</sup>, R<sup>9</sup> and R<sup>10</sup>, and R<sup>10</sup> and R<sup>11</sup> together 10 form an alkenylene chain completing a 5 or 6-membered aromatic ring, which ring may optionally include one or more divalent nitrogen, sulfur or oxygen atoms; and

(Va)



(Vb)



(Vc)



(Vd)



(Ve)



(Vf)



(Vg)



IV(a)

35

IV(b)

40

45

50

(V)

55



wherein:

Q is S or NR<sup>6</sup>;R<sup>6</sup> is hydrogen or alkyl;

R<sup>8</sup>, R<sup>9</sup>, R<sup>10</sup> and R<sup>11</sup> are independently selected so as to be the same or different at each occurrence and are selected from hydrogen, alkyl, alkenyl, alkoxy, alkanoyl, 65 alkylthio, aryloxy, alkylthioalkyl, alkylaryl, arylalkyl, amino, alkylamino, dialkylamino, aryl, alkylsulfinyl,

wherein:

Q is S or NH; and

T is the same or different at each occurrence and is selected from 5, NR<sup>6</sup>, O, SiR<sup>6</sup><sub>2</sub>, Se, and PR<sup>6</sup>;

R<sup>6</sup> is hydrogen or alkyl.

7. An electrically conductive polymer composition of claim 2 wherein the polycyclic heteroaromatics have structure represented by Formula VI:



(VI)

wherein:

Q is S or NR<sup>6</sup>;

T is selected from S, NR<sup>6</sup>, O, SiR<sup>6</sup><sub>2</sub>, Se, and PR<sup>6</sup>;

E is selected from alkenylene, arylene, and heteroarylene;

R<sup>6</sup> is hydrogen or alkyl;

R<sup>12</sup> is the same or different at each occurrence and is selected from hydrogen, alkyl, alkenyl, alkoxy, alkanoyl, alkythio, aryloxy, alkylthioalkyl, alkylaryl, arylalkyl, amino, alkylamino, dialkylamino, aryl, alkylsulfinyl, alkoxyalkyl, alkylsulfonyl, arylthio, arylsulfinyl, alkoxy carbonyl, arylsulfonyl, acrylic acid, phosphoric acid, phosphonic acid, halogen, nitro, nitrile, cyano, hydroxyl, epoxy, silane, siloxane, alcohol, benzyl, carboxylate, ether, ether carboxylate, amidosulfonate, ether sulfonate, ester sulfonate, and urethane; or two R<sup>12</sup> groups together may form an alkylene or alkenylene chain completing a 3, 4, 5, 6, or 7-membered aromatic or alicyclic ring, which ring may optionally include one or more divalent nitrogen, sulfur or oxygen atoms.

8. An electrically conductive polymer composition of claim 1 wherein each second electrically conductive polymer comprises one or more independently substituted or unsubstituted monomers selected from alkenyls, alkynyls, arylenes, and heteroarylenes.

9. An electrically conductive polymer composition of claim 8 wherein the independently substituted or unsubstituted monomers are selected from fluorene, oxadiazoles, thiadiazole, benzothiadiazoles, phenylenevinylenes, phenyleneethynylenes, pyridine, diazines, and triazines.

10. An electrically conductive polymer composition of claim 1 wherein the organic solvent wettable fluorinated acid polymer has a backbone selected from polyolefins, polyacrylates, polymethacrylates, polyimides, polyamides, polyaramids, polyacrylamides, polystyrenes, and copolymers thereof.

11. An electrically conductive polymer composition of claim 10 wherein the fluorinated acid polymer backbone is fluorinated.

12. An electrically conductive polymer composition of claim 11 wherein the fluorinated acid polymer has fluorinated pendant groups selected from ether sulfonates, ester sulfonates, and ether sulfonimides.

13. An electrically conductive polymer composition of claim 10 wherein the fluorinated acid polymer comprises one or more independently substituted or unsubstituted monomers selected from styrene sulfonic acids or sulfonated ether

sulfones, trifluorostyrene sulfonates, sulfonimides, perfluoroalkyl sulfonate ethers, fused polycyclic fluorinated acids, and perfluoroalkyl sulfonic acid ethers.

14. An electrically conductive polymer composition of claim 13 wherein the styrene sulfonic acids or sulfonated ether sulfones have structure represented by Formula VII:



(VII)

where:

20 b is an integer from 1 to 5;

R<sup>13</sup> is OH or NHR<sup>14</sup>, and

R<sup>14</sup> is alkyl, fluoroalkyl, sulfonylalkyl, or sulfonylfluoroalkyl.

15. An electrically conductive polymer composition of claim 13 wherein the trifluorostyrene sulfonates have structure represented by Formula VIII:



(VIII)

where:

W is selected from (CF<sub>2</sub>)<sub>q</sub>, O(CF<sub>2</sub>)<sub>q</sub>, S(CF<sub>2</sub>)<sub>q</sub>, (CF<sub>2</sub>)<sub>q</sub>O(CF<sub>2</sub>)<sub>q</sub>, and SO<sub>2</sub>(CF<sub>2</sub>)<sub>q</sub>,

b is independently an integer from 1 to 5;

R<sup>13</sup> is OH or NHR<sup>14</sup>, and

R<sup>14</sup> is alkyl, fluoroalkyl, sulfonylalkyl, or sulfonylfluoroalkyl. In one embodiment, the monomer containing W equal to S(CF<sub>2</sub>)<sub>q</sub> is polymerized then oxidized to give the polymer containing W equal to SO<sub>2</sub>(CF<sub>2</sub>)<sub>q</sub>.

16. An electrically conductive polymer composition of claim 13 wherein the sulfonimides have structure represented by Formula IX:



(IX)

where:

R<sub>f</sub> is selected from fluorinated alkenylene, fluorinated heteroalkylene, fluorinated arylene, or fluorinated heteroarylene;

R<sub>g</sub> is selected from fluorinated alkenylene, fluorinated heteroalkylene, fluorinated arylene, fluorinated heteroarylene, arylene, or heteroarylene; and

n is at least 4.

17. An electrically conductive polymer composition of claim 13 wherein the perfluoroalkyl sulfonate ethers have structure represented by Formula XI:



where:

R<sup>16</sup> is a fluorinated alkyl or a fluorinated aryl group;

a, b, c, d, and e are each independently 0 or an integer from 1 to 4; and

n is at least 4.

18. An electrically conductive polymer composition of claim 13 wherein the fused polycyclic fluorinated acids have structure represented by formulas selected from Formula XII 20 and Formulas XIIa-XIId:



wherein d is 0, 1, or 2;

R<sup>17</sup> to R<sup>20</sup> are independently H, halogen, alkyl or alkoxy of 1 to 10 carbon atoms, Y, C(R<sub>f</sub>)(R<sub>f</sub>)OR<sup>21</sup>, R<sup>4</sup>Y or OR<sup>4</sup>Y; Y is COE<sup>2</sup>, SO<sub>2</sub>E<sup>2</sup>, or sulfonimide;

R<sup>21</sup> is hydrogen or an acid-labile protecting group;

R<sub>f</sub> is the same or different at each occurrence and is a fluoroalkyl group of 1 to 10 carbon atoms, or taken together are (CF<sub>2</sub>)<sub>e</sub> where e is 2 to 10;

R<sup>4</sup> is an alkylene group;

E<sup>2</sup> is OH, halogen, or OR<sup>7</sup>; and

R<sup>5</sup> is an alkyl group;

with the proviso that at least one of R<sup>17</sup> to R<sup>20</sup> is Y, R<sup>4</sup>Y or OR<sup>4</sup>Y, R<sup>4</sup>, R<sup>5</sup>, and R<sup>17</sup> to R<sup>20</sup> may optionally be substituted by halogen or ether oxygen; and

(XII)

25

30

35

40

45

50

(XI)

-continued

(XIId)



wherein R<sup>21</sup> is a group capable of forming or rearranging to a tertiary cation, more typically an alkyl group of 1 to 20 carbon atoms, and most typically t-butyl.

19. An electrically conductive polymer composition of claim 1 wherein the organic solvent non-wettable fluorinated acid polymer comprises polymeric acids comprising functional groups selected from carboxylic, sulfonic, phosphoric, and phosphonic acid groups and sulfonimides, including combinations thereof.

20. An electrically conductive polymer composition of claim 19 wherein the functional groups are present on the polymeric backbone, sides chains, pendant groups, or combinations thereof.

21. An electrically conductive polymer composition of claim 20 wherein the pendant groups comprise siloxane sulfonic acid.

22. An electrically conductive polymer composition of claim 20 wherein the pendant groups comprise groups selected from structures represented by Formula XIV and Formula XV:



(XIV)

wherein R<sub>f</sub><sup>2</sup> is F or a perfluoroalkyl radical having 1-10 carbon atoms either unsubstituted or substituted by one or more ether oxygen atoms, h=0 or 1, i=0 to 3, and g=0 or 1; and

(XIIa)

(XV)



where j≥0, k≥0 and 4≤(j+k)≤199, Q1 and Q2 are F or H, R<sub>f</sub><sup>2</sup> is F or a perfluoroalkyl radical having 1-10 carbon atoms either unsubstituted or substituted by one or more ether oxygen atoms, h=0 or 1, i=0 to 3, g=0 or 1, and E4 is H or an alkali metal.

23. An electrically conductive polymer composition of claim 19 wherein the fluorinated acid polymer is a colloid-forming polymeric acid.



(XIIb)

(XV)



(XIIc)



**41**

**24.** An electrically conductive polymer composition of claim **23** wherein the fluorinated acid polymer comprises an FSA polymer.

**25.** An electrically conductive polymer composition of claim **1** comprising a buffer.

**42**

**26.** An electronic device comprising an electrically conductive polymer composition of claim **1**.

\* \* \* \* \*